



US011692281B2

(12) **United States Patent**  
**Lomasney**

(10) **Patent No.:** **US 11,692,281 B2**  
(45) **Date of Patent:** **Jul. 4, 2023**

(54) **METHOD AND APPARATUS FOR  
CONTINUOUSLY APPLYING  
NANOLAMINATE METAL COATINGS**

(71) Applicant: **Modumetal, Inc.**, Seattle, WA (US)

(72) Inventor: **Christina A. Lomasney**, Seattle, WA (US)

(73) Assignee: **Modumetal, Inc.**, Seattle, WA (US)

(\*) Notice: Subject to any disclaimer, the term of this patent is extended or adjusted under 35 U.S.C. 154(b) by 0 days.

(21) Appl. No.: **16/582,931**

(22) Filed: **Sep. 25, 2019**

(65) **Prior Publication Data**

US 2020/0283923 A1 Sep. 10, 2020

**Related U.S. Application Data**

(60) Division of application No. 15/464,245, filed on Mar. 20, 2017, now Pat. No. 10,472,727, which is a (Continued)

(51) **Int. Cl.**

*C25D 17/00* (2006.01)  
*C25D 21/10* (2006.01)  
*C25D 5/10* (2006.01)  
*C25D 5/12* (2006.01)  
*C25D 5/18* (2006.01)  
*C25D 5/34* (2006.01)  
*C25D 5/48* (2006.01)  
*C25D 5/56* (2006.01)  
*C25D 7/04* (2006.01)

(Continued)

(52) **U.S. Cl.**

CPC ..... *C25D 21/10* (2013.01); *C25D 5/10* (2013.01); *C25D 5/12* (2013.01); *C25D 5/14* (2013.01); *C25D 5/18* (2013.01); *C25D 5/34* (2013.01); *C25D 5/48* (2013.01); *C25D 5/56* (2013.01)

(2013.01); *C25D 5/617* (2020.08); *C25D 7/04* (2013.01); *C25D 7/0607* (2013.01); *C25D 17/00* (2013.01); *C25D 17/02* (2013.01); *C25D 21/12* (2013.01); *C23C 18/1653* (2013.01)

(58) **Field of Classification Search**

None  
See application file for complete search history.

(56) **References Cited**

U.S. PATENT DOCUMENTS

1,733,404 A 10/1929 Fahrenwald  
1,982,009 A 11/1934 McKinney et al.  
(Continued)

FOREIGN PATENT DOCUMENTS

CN 1236024 A 11/1999  
CN 1380446 A 11/2002  
(Continued)

OTHER PUBLICATIONS

“Appendix 1: Literature review (Task 1): Literature review concerning the improvement of galvanneal (GA) coating adherence during shear test of adhesively bonded GA steel sheets,” 70 pages, no date.

(Continued)

*Primary Examiner* — Stefanie S Wittenberg

(74) *Attorney, Agent, or Firm* — Seed IP Law Group LLP

(57) **ABSTRACT**

Described herein are apparatus and methods for the continuous application of nanolaminated materials by electrodeposition.

**18 Claims, 11 Drawing Sheets**



| Related U.S. Application Data                                              |                |                           |
|----------------------------------------------------------------------------|----------------|---------------------------|
| continuation of application No. PCT/US2015/050932, filed on Sep. 18, 2015. | 4,652,348 A    | 3/1987 Yahalom et al.     |
| (60) Provisional application No. 62/052,345, filed on Sep. 18, 2014.       | 4,666,567 A    | 5/1987 Loch               |
| (51) Int. Cl.                                                              | 4,670,356 A    | 6/1987 Sato et al.        |
| <i>C25D 7/06</i> (2006.01)                                                 | 4,678,552 A    | 7/1987 Chen               |
| <i>C25D 17/02</i> (2006.01)                                                | 4,678,721 A    | 7/1987 den Broeder et al. |
| <i>C25D 21/12</i> (2006.01)                                                | 4,702,802 A    | 10/1987 Umino et al.      |
| <i>C25D 5/00</i> (2006.01)                                                 | H543 H         | 11/1988 Chen et al.       |
| <i>C25D 5/14</i> (2006.01)                                                 | 4,795,735 A    | 1/1989 Uiu et al.         |
| <i>C23C 18/16</i> (2006.01)                                                | 4,834,845 A    | 5/1989 Muko et al.        |
| (56) References Cited                                                      | 4,839,214 A    | 6/1989 Oda et al.         |
| U.S. PATENT DOCUMENTS                                                      | 4,869,971 A    | 9/1989 Nee et al.         |
| 2,428,033 A 9/1947 Nachtman                                                | 4,885,215 A    | 12/1989 Yoshioka et al.   |
| 2,436,316 A 2/1948 Lum et al.                                              | 4,904,542 A    | 2/1990 Mroczkowski        |
| 2,470,775 A 5/1949 Jemstedt et al.                                         | 4,904,543 A    | 2/1990 Sakakima et al.    |
| 2,558,090 A 6/1951 Jemstedt                                                | 4,909,917 A    | 3/1990 Harrison et al.    |
| 2,642,654 A 6/1953 Ahrens                                                  | 4,923,574 A    | 5/1990 Cohen              |
| 2,678,909 A 5/1954 Jemstedt et al.                                         | 4,975,337 A    | 12/1990 Hyner et al.      |
| 2,694,743 A 11/1954 Ruskin et al.                                          | 5,043,230 A    | 8/1991 Jagannathan et al. |
| 2,706,170 A 4/1955 Marchese                                                | 5,045,356 A    | 9/1991 Uemura et al.      |
| 2,891,309 A 6/1959 Fenster                                                 | 5,056,936 A    | 10/1991 Mahrus et al.     |
| 3,090,733 A 5/1963 Brown                                                   | 5,059,493 A    | 10/1991 Takahata          |
| 3,255,781 A 6/1966 Gillespie, Jr.                                          | 5,073,237 A    | 12/1991 Bacher et al.     |
| 3,282,810 A 11/1966 Odekerken                                              | 5,079,039 A    | 1/1992 Heraud et al.      |
| 3,355,374 A * 11/1967 Brewer .....                                         | C25D 13/22     | 5,096,564 A               |
|                                                                            | 204/489        | 3/1992 Jowitt et al.      |
| 3,359,469 A 12/1967 Levy et al.                                            | 5,156,729 A    | 10/1992 Mahrus et al.     |
| 3,362,851 A 1/1968 Dunster                                                 | 5,156,899 A    | 10/1992 Kistrup et al.    |
| 3,483,113 A 12/1969 Carter                                                 | 5,158,653 A    | 10/1992 Lashmore et al.   |
| 3,549,505 A 12/1970 Hanusa                                                 | 5,190,637 A    | 3/1993 Guckel             |
| 3,616,286 A 10/1971 Aylward et al.                                         | 5,228,967 A    | 7/1993 Crites et al.      |
| 3,633,520 A 1/1972 Stiglich, Jr.                                           | 5,234,562 A    | 8/1993 Uenishi et al.     |
| 3,669,865 A * 6/1972 Semienko .....                                        | C25D 7/0607    | 5,268,235 A               |
|                                                                            | 204/207        | 12/1993 Lashmore et al.   |
| 3,673,073 A 6/1972 Tobey et al.                                            | 5,300,165 A    | 4/1994 Sugikawa           |
| 3,716,464 A 2/1973 Kovac et al.                                            | 5,320,719 A    | 6/1994 Lasbmore et al.    |
| 3,753,664 A 8/1973 Klingenmaier et al.                                     | 5,326,454 A    | 7/1994 Engelhaupt         |
| 3,759,799 A 9/1973 Reinke                                                  | 5,352,266 A    | 10/1994 Erb et al.        |
| 3,787,244 A 1/1974 Schulmeister et al.                                     | 5,364,523 A    | 11/1994 Tanaka et al.     |
| 3,866,289 A 2/1975 Brown et al.                                            | 5,378,583 A    | 1/1995 Guckel et al.      |
| 3,941,674 A 5/1976 Vanmunster                                              | 5,413,874 A    | 5/1995 Moysan, III et al. |
| 3,994,694 A 11/1976 Clauss et al.                                          | 5,431,800 A    | 7/1995 Kirchhoff et al.   |
| 3,996,114 A 12/1976 Ehrsam                                                 | 5,461,769 A    | 10/1995 McGregor          |
| 4,053,371 A 10/1977 Towsley                                                | 5,472,795 A    | 12/1995 Atita             |
| 4,105,526 A 8/1978 Lewellen, Jr. et al.                                    | 5,489,488 A    | 2/1996 Asai et al.        |
| 4,107,003 A 8/1978 Anselrode                                               | 5,500,600 A    | 3/1996 Moyes              |
| 4,125,447 A 11/1978 Bachert                                                | 5,547,096 A    | 4/1996 Kleyn              |
| 4,191,617 A 3/1980 Hurley et al.                                           | 5,527,445 A    | 6/1996 Palumbo            |
| 4,204,918 A 5/1980 McIntyre et al.                                         | 5,545,435 A    | 8/1996 Steffier           |
| 4,216,272 A 8/1980 Clauss                                                  | 5,620,800 A    | 4/1997 De Leeuw et al.    |
| 4,246,057 A 1/1981 Janowski et al.                                         | 5,660,704 A    | 8/1997 Murase             |
| 4,269,672 A 5/1981 Inoue                                                   | 5,679,232 A    | 10/1997 Fedor et al.      |
| 4,284,688 A 8/1981 Stücheli et al.                                         | 5,738,951 A    | 4/1998 Goujard et al.     |
| 4,314,893 A 2/1982 Clauss                                                  | 5,742,471 A    | 4/1998 Barbee, Jr. et al. |
| 4,405,427 A 9/1983 Byrd                                                    | 5,775,402 A    | 7/1998 Sachs et al.       |
| 4,422,907 A 12/1983 Birkmaier et al.                                       | 5,783,259 A    | 7/1998 McDonald           |
| 4,461,680 A 7/1984 Lashmore                                                | 5,798,033 A    | 8/1998 Uemiya et al.      |
| 4,464,232 A 8/1984 Wakano et al.                                           | 5,800,930 A    | 9/1998 Chen et al.        |
| 4,510,209 A 4/1985 Hada et al.                                             | 5,828,526 A    | 10/1998 Kagawa et al.     |
| 4,519,878 A 5/1985 Hara et al.                                             | 5,912,069 A    | 6/1999 Yializis et al.    |
| 4,529,492 A 7/1985 Buchholz et al.                                         | 5,930,085 A    | 7/1999 Kitade et al.      |
| 4,540,472 A 9/1985 Johnson et al.                                          | 5,942,096 A    | 8/1999 Ruzicka et al.     |
| 4,543,300 A 9/1985 Hara et al.                                             | 5,952,111 A    | 9/1999 Sugg et al.        |
| 4,543,803 A 10/1985 Keyasko                                                | 5,958,604 A *  | 9/1999 Riabkov .....      |
| 4,591,418 A 5/1986 Snyder                                                  | C25D 5/611     | 205/148                   |
| 4,592,808 A 6/1986 Doubt                                                   | 6,036,832 A    | 3/2000 Knol et al.        |
| 4,597,836 A 7/1986 Schaer et al.                                           | 6,036,833 A    | 3/2000 Tang et al.        |
| 4,613,388 A 9/1986 Walter et al.                                           | 6,071,398 A    | 6/2000 Martin et al.      |
| 4,620,661 A 11/1986 Slatterly                                              | 6,143,424 A    | 11/2000 Jonte et al.      |
|                                                                            | 6,143,430 A    | 11/2000 Miyasaka et al.   |
|                                                                            | 6,193,858 B1   | 2/2001 Hradil et al.      |
|                                                                            | 6,200,452 B1 * | 3/2001 Angelini .....     |
|                                                                            | C25D 7/04      | 204/198                   |
|                                                                            | 6,203,936 B1   | 3/2001 Cisar et al.       |
|                                                                            | 6,212,078 B1   | 4/2001 Hunt et al.        |
|                                                                            | 6,214,473 B1   | 4/2001 Hunt et al.        |
|                                                                            | 6,284,357 B1   | 9/2001 Lackey et al.      |
|                                                                            | 6,312,579 B1   | 11/2001 Bank et al.       |
|                                                                            | 6,344,123 B1   | 2/2002 Bhatnagar          |
|                                                                            | 6,355,153 B1   | 3/2002 Uzoh et al.        |
|                                                                            | 6,398,937 B1 * | 6/2002 Menini .....       |
|                                                                            | C25D 5/20      | 205/125                   |

| (56)                  | References Cited |                       |                  |         |                           |            |  |
|-----------------------|------------------|-----------------------|------------------|---------|---------------------------|------------|--|
| U.S. PATENT DOCUMENTS |                  |                       |                  |         |                           |            |  |
| 6,409,907 B1          | 6/2002           | Braun et al.          | 2004/0027715 A1  | 2/2004  | Hixson-Goldsmith et al.   |            |  |
| 6,415,942 B1          | 7/2002           | Fenton et al.         | 2004/0031691 A1  | 2/2004  | Kelly et al.              |            |  |
| 6,461,678 B1          | 10/2002          | Chen et al.           | 2004/0067314 A1  | 4/2004  | Joshi et al.              |            |  |
| 6,466,417 B1          | 10/2002          | Gill                  | 2004/0154925 A1  | 8/2004  | Podlaha et al.            |            |  |
| 6,468,672 B1          | 10/2002          | Donovan, III et al.   | 2004/0178076 A1  | 9/2004  | Stonas et al.             |            |  |
| 6,482,298 B1          | 11/2002          | Bhatnagar             | 2004/0211672 A1  | 10/2004 | Ishigami et al.           |            |  |
| 6,537,683 B1          | 3/2003           | Staschko et al.       | 2004/0232005 A1  | 11/2004 | Hubel                     |            |  |
| 6,547,944 B2          | 4/2003           | Schreiber et al.      | 2004/0234683 A1  | 11/2004 | Tanaka et al.             |            |  |
| 6,592,739 B1          | 7/2003           | Sonoda et al.         | 2004/0239836 A1  | 12/2004 | Chase                     |            |  |
| 6,725,916 B2          | 4/2004           | Gray et al.           | 2005/0002228 A1  | 1/2005  | Diény et al.              |            |  |
| 6,739,028 B2          | 5/2004           | Sievenpiper et al.    | 2005/0109433 A1  | 5/2005  | Danger et al.             |            |  |
| 6,777,831 B2          | 8/2004           | Gutiérrez, Jr. et al. | 2005/0205425 A1  | 9/2005  | Palumbo et al.            |            |  |
| 6,800,121 B2          | 10/2004          | Shahin                | 2005/0221100 A1  | 10/2005 | Kirihara et al.           |            |  |
| 6,884,499 B2          | 4/2005           | Penich et al.         | 2005/0279640 A1  | 12/2005 | Shimoyama et al.          |            |  |
| 6,902,827 B2          | 6/2005           | Kelly et al.          | 2006/0065533 A1* | 3/2006  | Inoue .....               | C25D 3/38  |  |
| 6,908,667 B2          | 6/2005           | Christ et al.         |                  |         |                           | 205/81     |  |
| 6,923,898 B2          | 8/2005           | Yoshimura et al.      | 2006/0135281 A1  | 6/2006  | Palumbo et al.            |            |  |
| 6,979,490 B2          | 12/2005          | Steffier              | 2006/0135282 A1  | 6/2006  | Palumbo et al.            |            |  |
| 7,285,202 B2          | 10/2007          | Rumpf                 | 2006/0201817 A1  | 9/2006  | Guggemos et al.           |            |  |
| 7,581,933 B2          | 9/2009           | Bruce et al.          | 2006/0243597 A1  | 11/2006 | Matefi-Tempfli et al.     |            |  |
| 7,632,590 B2          | 12/2009          | Punsalan et al.       | 2006/0269770 A1  | 11/2006 | Cox et al.                |            |  |
| 7,736,753 B2          | 6/2010           | Deligianni et al.     | 2006/0272949 A1  | 12/2006 | Detor et al.              |            |  |
| 8,084,564 B2          | 12/2011          | Kano et al.           | 2006/0286348 A1  | 12/2006 | Sauer                     |            |  |
| 8,128,752 B2          | 3/2012           | Kim                   | 2007/0158204 A1  | 7/2007  | Taylor et al.             |            |  |
| 8,152,985 B2          | 4/2012           | Macary                | 2007/0269648 A1  | 11/2007 | Schuh et al.              |            |  |
| 8,177,945 B2          | 5/2012           | Arvin et al.          | 2007/0278105 A1  | 12/2007 | Ettel                     |            |  |
| 8,192,608 B2          | 6/2012           | Matthews              | 2008/0063866 A1  | 3/2008  | Allen et al.              |            |  |
| 8,253,035 B2          | 8/2012           | Matsumoto             | 2008/0093221 A1  | 4/2008  | Basol                     |            |  |
| 8,293,077 B2          | 10/2012          | Vacheron              | 2008/0102360 A1  | 5/2008  | Stimits et al.            |            |  |
| 8,585,875 B2          | 11/2013          | Cummings et al.       | 2008/0226976 A1  | 9/2008  | Stimits                   |            |  |
| 8,617,456 B1          | 12/2013          | Pechenik et al.       | 2008/0245669 A1  | 10/2008 | Yoshioka et al.           |            |  |
| 8,814,437 B2          | 8/2014           | Braun                 | 2008/0271995 A1  | 11/2008 | Savastiouk et al.         |            |  |
| 8,871,065 B2          | 10/2014          | Vacheron              | 2008/0283236 A1  | 11/2008 | Akers et al.              |            |  |
| 8,916,001 B2          | 12/2014          | Pryce Lewis et al.    | 2009/0004465 A1  | 1/2009  | Kano et al.               |            |  |
| 9,005,420 B2          | 4/2015           | Tomantschger et al.   | 2009/0101511 A1  | 4/2009  | Lochman et al.            |            |  |
| 9,056,405 B2          | 6/2015           | Sato et al.           | 2009/0114530 A1* | 5/2009  | Noda .....                | C25D 17/12 |  |
| 9,080,692 B2          | 7/2015           | Tomomori et al.       |                  |         |                           | 204/230.2  |  |
| 9,108,506 B2          | 8/2015           | Whitaker et al.       | 2009/0155617 A1  | 6/2009  | Tholen et al.             |            |  |
| 9,115,439 B2          | 8/2015           | Whitaker              | 2009/0283410 A1  | 11/2009 | Whitaker                  |            |  |
| 9,234,294 B2          | 1/2016           | Whitaker et al.       | 2010/0078330 A1  | 4/2010  | Nagai et al.              |            |  |
| 9,273,932 B2          | 3/2016           | Whitaker et al.       | 2010/0116675 A1  | 5/2010  | Kim et al.                |            |  |
| 9,732,433 B2          | 8/2017           | Caldwell et al.       | 2010/0187117 A1  | 7/2010  | Sklar et al.              |            |  |
| 9,758,891 B2          | 9/2017           | Bao                   | 2010/0304063 A1  | 12/2010 | Lingenfelter et al.       |            |  |
| 9,783,907 B2          | 10/2017          | Cai et al.            | 2010/0304179 A1  | 12/2010 | McCrea et al.             |            |  |
| 9,938,629 B2          | 4/2018           | Whitaker et al.       | 2010/0319757 A1  | 12/2010 | Facchini et al.           |            |  |
| 10,041,185 B2         | 8/2018           | Sukenari              | 2011/0111296 A1  | 12/2010 | Oetting                   |            |  |
| 10,253,419 B2         | 4/2019           | Lomasney              | 2011/0162970 A1  | 5/2011  | Bao                       |            |  |
| 10,266,957 B2         | 4/2019           | Sugawara et al.       | 2011/0180413 A1  | 7/2011  | Sato                      |            |  |
| 10,472,727 B2         | 11/2019          | Lomasney              | 2011/0186582 A1  | 8/2011  | Whitaker et al.           |            |  |
| 10,513,791 B2         | 12/2019          | Lomasney et al.       | 2011/0256356 A1  | 10/2011 | Whitaker                  |            |  |
| 10,544,510 B2         | 1/2020           | Lomasney              | 2011/0277313 A1  | 11/2011 | Tomantschger et al.       |            |  |
| 10,662,542 B2         | 5/2020           | Caldwell et al.       | 2012/0118745 A1  | 5/2012  | Soracco et al.            |            |  |
| 10,689,773 B2         | 6/2020           | Whitaker et al.       | 2012/0135270 A1  | 5/2012  | Berdichevsky et al.       |            |  |
| 10,695,797 B2         | 6/2020           | Andreae et al.        | 2012/0231574 A1  | 9/2012  | Wilbuer et al.            |            |  |
| 10,781,524 B2         | 9/2020           | Whitaker et al.       | 2012/0282417 A1  | 11/2012 | Wang                      |            |  |
| 10,808,322 B2         | 10/2020          | Whitaker et al.       | 2013/0052343 A1  | 2/2013  | Garcia et al.             |            |  |
| 10,844,504 B2         | 11/2020          | Sklar                 | 2013/0071755 A1  | 3/2013  | Dieny et al.              |            |  |
| 10,851,464 B1         | 12/2020          | Kobayashi et al.      | 2013/0075264 A1  | 3/2013  | Oguro                     |            |  |
| 10,961,635 B2         | 3/2021           | Whitaker              | 2013/0130057 A1  | 5/2013  | Cummings et al.           |            |  |
| 11,118,280 B2         | 9/2021           | Lomasney et al.       | 2013/0186852 A1  | 7/2013  | Caldwell et al.           |            |  |
| 11,168,408 B2         | 11/2021          | Sklar                 | 2013/0220831 A1  | 7/2013  | Dietrich et al.           |            |  |
| 11,180,864 B2         | 11/2021          | Lomasney              | 2013/0224008 A1  | 8/2013  | Dieny et al.              |            |  |
| 11,242,613 B2         | 2/2022           | Lomasney              | 2013/0323473 A1  | 8/2013  | Oguro                     |            |  |
| 11,286,575 B2         | 3/2022           | Lomasney et al.       | 2014/0163717 A1  | 12/2013 | Cheung et al.             |            |  |
| 11,293,272 B2         | 4/2022           | Lomasney              | 2014/0282417 A1  | 6/2014  | Vidaurre Heiremans et al. |            |  |
| 11,365,488 B2         | 6/2022           | Morgan et al.         | 2015/0315716 A1  | 6/2014  | Dietrich et al.           |            |  |
| 2001/0003384 A1       | 6/2001           | Morita                | 2015/0322588 A1  | 11/2015 | Rajagopalan et al.        |            |  |
| 2001/0037944 A1       | 11/2001          | Sanada et al.         | 2016/0002790 A1  | 1/2016  | Sherr et al.              |            |  |
| 2002/0011419 A1*      | 1/2002           | Arao .....            | C25D 9/08        | 205/333 | 11/2015                   | Whitaker   |  |
| 2002/0100858 A1       | 8/2002           | Weber                 | 2016/0002806 A1  | 1/2016  | Das et al.                |            |  |
| 2002/0179449 A1       | 12/2002          | Domeier et al.        | 2016/0002813 A1  | 6/2014  | Dietsch et al.            |            |  |
| 2003/0134142 A1       | 7/2003           | Ivey et al.           | 2016/0163717 A1  | 6/2014  | Rajagopalan et al.        |            |  |
| 2003/0234181 A1       | 12/2003          | Palumbo               | 2016/0221266 A1  | 8/2014  | Sherr et al.              |            |  |
| 2003/0236163 A1       | 12/2003          | Chaturvedi et al.     | 2016/0315716 A1  | 11/2015 | Whitaker                  |            |  |

(56)

## References Cited

## U.S. PATENT DOCUMENTS

|              |    |         |                            |
|--------------|----|---------|----------------------------|
| 2016/0159488 | A1 | 6/2016  | Roach et al.               |
| 2016/0160863 | A1 | 6/2016  | Roach et al.               |
| 2016/0214283 | A1 | 7/2016  | Schick et al.              |
| 2017/0016130 | A1 | 1/2017  | Testoni et al.             |
| 2017/0191177 | A1 | 7/2017  | Whitaker et al.            |
| 2017/0191179 | A1 | 7/2017  | Sklar                      |
| 2017/0275775 | A1 | 9/2017  | Guadarrama Calderon et al. |
| 2018/0016694 | A1 | 1/2018  | Bao                        |
| 2018/0066375 | A1 | 3/2018  | Morgan et al.              |
| 2018/0071980 | A1 | 3/2018  | Lomasney et al.            |
| 2018/0245229 | A1 | 8/2018  | Whitaker et al.            |
| 2019/0309430 | A1 | 10/2019 | Sklar                      |
| 2019/0360116 | A1 | 11/2019 | Collinson et al.           |
| 2020/0115998 | A1 | 4/2020  | Lomasney                   |
| 2020/0131658 | A1 | 4/2020  | Lomasney et al.            |
| 2020/0173032 | A1 | 6/2020  | Lomasney                   |
| 2020/0277706 | A1 | 9/2020  | Lomasney et al.            |
| 2020/0318245 | A1 | 10/2020 | Lomasney                   |
| 2020/0354846 | A1 | 11/2020 | Whitaker et al.            |
| 2020/0392642 | A1 | 12/2020 | Lomasney                   |
| 2021/0054522 | A1 | 2/2021  | Lomasney et al.            |
| 2021/0071303 | A1 | 3/2021  | Whitaker et al.            |
| 2021/0147995 | A1 | 5/2021  | Sklar                      |
| 2022/0081798 | A1 | 3/2022  | Collinson et al.           |
| 2022/0154357 | A1 | 5/2022  | Lomasney                   |

## FOREIGN PATENT DOCUMENTS

|    |                 |    |                         |
|----|-----------------|----|-------------------------|
| CN | 1924110         | A  | 3/2007                  |
| CN | 101113527       | A  | 1/2008                  |
| CN | 101195924       | A  | 6/2008                  |
| CN | 201857434       | *  | 6/2011 ..... C25D 7/06  |
| CN | 102148339       | A  | 8/2011                  |
| CN | 203584787       | U  | 5/2014                  |
| CN | 105442011       | A  | 3/2016                  |
| DE | 39 02 057       | A1 | 7/1990                  |
| DE | 10 2004 006 441 | A1 | 12/2005                 |
| DE | 10 2010 011 087 | A1 | 9/2011                  |
| EP | 1688518         | *  | 2/2006 ..... C25D 17/10 |
| EP | 2 189 554       | A1 | 5/2010                  |
| JP | S47-2005        | A  | 2/1972                  |
| JP | S47-33925       | A  | 11/1972                 |
| JP | S52-109439      | A  | 9/1977                  |
| JP | 58-197292       | A  | 11/1983                 |
| JP | S60-97774       | A  | 5/1985                  |
| JP | S61-99692       | A  | 5/1986                  |
| JP | H01-132793      | A  | 5/1989                  |
| JP | 2-214618        | A  | 8/1990                  |
| JP | H05-251849      | A  | 9/1993                  |
| JP | H06-196324      | A  | 7/1994                  |
| JP | 07-065347       | A  | 3/1995                  |
| JP | H09-119000      | A  | 5/1997                  |
| JP | 2000-239888     | A  | 9/2000                  |
| JP | 2001-152388     | A  | 6/2001                  |
| JP | 2001-181893     | A  | 7/2001                  |
| JP | 2002-53999      | A  | 2/2002                  |
| JP | 2006-035176     | A  | 2/2006                  |
| JP | 2009-215590     | A  | 9/2009                  |
| KR | 2003-0092463    | A  | 12/2003                 |
| KR | 20090068670     | *  | 6/2009 ..... C25D 17/00 |
| KR | 20-2010-0009670 | U  | 10/2010                 |
| KR | 20100009670     | *  | 10/2010 ..... C25D 5/14 |
| KR | 10-2015-0132043 | A  | 11/2015                 |
| SU | 36121           | A1 | 4/1934                  |
| WO | 83/02784        | A1 | 8/1983                  |
| WO | 95/14116        | A1 | 5/1995                  |
| WO | 2004/001100     | A1 | 12/2003                 |
| WO | 2007/045466     | A1 | 4/2007                  |
| WO | 2007/138619     | A1 | 12/2007                 |
| WO | 2008/057401     | A2 | 5/2008                  |
| WO | 2009/045433     | A1 | 4/2009                  |
| WO | 2011/033775     | A1 | 3/2011                  |
| WO | 2012/145750     | A2 | 10/2012                 |
| WO | 2013/133762     | A1 | 9/2013                  |
| WO | 2017/097300     | A1 | 6/2017                  |

## OTHER PUBLICATIONS

- “Low-temperature iron plating,” web blog article found at [http://blog.sina.com.cn/s/blog\\_48ed0a9c01100024z.html](http://blog.sina.com.cn/s/blog_48ed0a9c01100024z.html), published Mar. 22, 2006, 3 pages, (with English translation).
- Adams et al., “Controlling strength and toughness of multilayer films: A new multiscalar approach,” *J. Appl. Phys.* 74(2):1015-1021, 1993.
- Aizenberg et al., “Skeleton of *Euplectella* sp.: Structural Hierarchy from the Nanoscale to the Macroscale,” *Science* 309:215-218, 2005.
- Alfantazi et al., “Synthesis of nanocrystalline Zn—Ni alloy coatings,” *JMSLD 5* 15(15):1361-1363, 1996.
- Atanassov et al., “Electrodeposition and properties of nickel-manganese layers,” *Surface and Coatings Technology* 78:144-149, 1996.
- Bakonyi et al., “Electrodeposited multilayer films with giant magnetoresistance (GMR): Progress and problems,” *Progress in Materials Science* 55:107-245, 2010.
- Bartlett et al., “Electrochemical deposition of macroporous platinum, palladium and cobalt films using polystyrene latex sphere templates,” *Chem. Commun.*, pp. 1671-1672, 2000.
- Beattie et al., “Comparison of Electrodeposited Copper-Zinc Alloys Prepared Individually and Combinatorially,” *J. Electrochem. Soc.* 150(11):C802-C806, 2003.
- Bird et al., “Giant Magnetoresistance in Electrodeposited Ni/Cu and Co/Cu Multilayers,” *J. Electrochem. Soc.* 142(4):L65-L66, 1995.
- Blum, “The Structure and Properties of Alternately Electrodeposited Metals,” presented at the Fortieth General Meeting of the American Electrochemical Society, Lake Placid, New York, Oct. 1, 1921, 14 pages.
- Cohen et al., “Electroplating of Cyclic Multilayered Alloy (CMA) Coatings,” *J. Electrochem. Soc.* 130(10):1987-1995, 1983.
- Cowles, “High cycle fatigue in aircraft gas turbines—an industry perspective,” *International Journal of Fracture* 80(2-3):147-163, 1996.
- “Designing with Metals: Dissimilar Metals and The Galvanic Series,” printed Oct. 5, 2017, 3 pages.
- Despic et al., “Electrochemical Formation of Laminar Deposits of Controlled Structure and Composition,” *J. Electrochem. Soc.* 136(6):1651-1657, 1989.
- Dini et al. “On the High Temperature Ductility Properties of Electrodeposited Sulfamate Nickel,” *Plating and Surface Finishing* 65(2):36-40, 1978.
- Eтminanfar et al., “Corrosion resistance of multilayer coatings of nanolayered Cr/Ni electrodeposited from Cr(III)—Ni(II) bath,” *Thin Solid Films* 520:5322-5321, 2012.
- Gasser et al., “Materials Design for Acoustic Liners: an Example of Tailored Multifunctional Materials,” *Advanced Engineering Materials* 6(1-2):97-102, 2004.
- Georgescu et al., “Magnetic Behavior of [Ni/Co—Ni—Mg—N] x n Cylindrical Multilayers prepared by Magnetoelectrolysis,” *Phys. Stat. Sol. (a)* 189(3):1051-1055, 2002.
- Ghanem et al., “A double templated electrodeposition method for the fabrication of arrays of metal nanodots,” *Electrochemistry Communications* 6:447-453, 2004.
- Grimmett et al., “Pulsed Electrodeposition of Iron-Nickel Alloys,” *J. Electrochem. Soc.* 137(11):3414-3418, 1990.
- Hariyanti, “Electroplating of Cu—Sn Alloys and Compositionally Modulated Multilayers of Cu—Sn—Zn—Ni Alloys on Mild Steel Substrate,” Master of Science Thesis, University of Science, Malaysia, Penang, Malaysia, 2007.
- Harris et al., “Improved Single Crystal Superalloys, CMSX-4® (SLS)[La+Y] and CMSX-486®,” *TMS (The Minerals, Metals & Materials Society), Superalloys*, p. 45-52, 2004.
- Huang et al., “Hardness variation and annealing behavior of a Cr—Ni multilayer electroplated in a trivalent chromium-based bath,” *Surface and Coatings Technology* 203:3320-3324, 2009.
- Huang et al., “Characterization of Cr—Ni multilayers electroplated from a chromium(III)-nickel(II) bath using pulse current,” *Scripta Materialia*, 57:61-64, 2007.

(56)

## References Cited

## OTHER PUBLICATIONS

- Igawa et al., "Fabrication of SiC fiber reinforced SiC composite by chemical vapor infiltration for excellent mechanical properties," *Journal of Physics and Chemistry of Solids* 66:551-554, 2005.
- Ivanov et al., "Corrosion resistance of compositionally modulated multilayered Zn—Ni alloys deposited from a single bath," *Journal of Applied Electrochemistry* 33:239-244, 2003.
- Jeong et al., "The Effect of Grain Size on the Wear Properties of Electrodeposited Nanocrystalline Nickel Coatings," *Scripta Mater.* 44:493-499, 2001.
- Jia et al., "LIGA and Micromolding" Chapter 4, *The MEMS Handbook*, 2nd edition, CRC Press, Boca Raton, Florida, Edited by Mohamed Gad-el-Hak, 2006.
- Kalu et al., "Cyclic voltammetric studies of the effects of time and temperature on the capacitance of electrochemically deposited nickel hydroxide," *Journal of Power Sources* 92:163-167, 2001.
- Kaneko et al., "Vickers hardness and deformation of Ni/Cu nanomultilayers electrodeposited on copper substrates," Eleventh International Conference on Intergranular and Interphase Boundaries 2004, *Journal of Material Science* 40:3231-3236, 2005.
- Karimpoor et al., "Tensile Properties of Bulk Nanocrystalline Hexagonal Cobalt Electrodeposits", *Materials Science Forum* 386-388:415-420, 2002.
- Keckes et al., "Cell-wall recovery after irreversible deformation of wood," *Nature Materials* 2:810-814, 2003.
- Kirilova et al., "Corrosion behaviour of Zn—Co compositionally modulated multilayers electrodeposited from single and dual baths," *Journal of Applied Electrochemistry* 29:1133-1137, 1999.
- Kockar et al., "Effect of potentiostatic waveforms on properties of electrodeposited NiFe alloy films," *Eur. Phys. J. B*(42):497-501, 2004.
- Kruth et al., "Progress in Additive Manufacturing and Rapid Prototyping" *CIRP Annals* 47(2):525-540, 1998.
- Lashmore et al., "Electrodeposited Cu—Ni Textured Superlattices," *J. Electrochem. Soc.* 135(5)A218-1221, 1988.
- Lashmore et al., "Electrodeposited Multilayer Metallic Coatings", *Encyclopedia of Materials Science and Engineering*, Supp. vol. 1:136-140, 1988.
- Leisner et al., "Methods for electrodepositing composition-modulated alloys," *Journal of Materials Processing Technology* 58:39-44, 1996.
- Leith et al., "Characterization of Flow-Induced Compositional Structure in Electrodeposited NiFe Composition-Modulated Alloys" *J. Electrochem. Soc.* 145(8):2821-2833, 1998.
- Lekka et al., "Corrosion and wear resistant electrodeposited composite coatings," *Electrochimica Acta* 50:4551-4556, 2005.
- Lewis et al., "Stability in thin film multilayers and microlaminates: the role of free energy, structure, and orientation at interfaces and grain boundaries," *Scripta Materialia* 48:1079-1085, 2003.
- Low et al., "Electrodeposition of composite coatings containing nanoparticles in a metal deposit," *Surface & Coating Technology* 201:311-383, 2006.
- Malone, "New Developments in Electroformed Nickel-Based Structural Alloys," *Plating and Surface Finishing* 74(1):50-56, 1987.
- Marchese, "Stress Reduction of Electrodeposited Nickel," *Journal of the Electrochemical Society* 99(2):39-43, 1952.
- Meng et al., "Fractography, elastic modulus, and oxidation resistance of Novel metal-intermetallic Ni/Ni<sub>3</sub>Al multilayer films," *J. Mater. Res.* 17(4):190-196, 2002.
- Naslain et al., "Synthesis of highly tailored ceramic matrix composites by pressure-pulsed CVI," *Solid State Ionics* 747-742:541-548, 2001.
- Naslain, "The design of the fibre-matrix interfacial zone in ceramic matrix composites," *Composites Part A* 29A:1145-1155, 1998.
- Nicholls, "Advances in Coating Design for High-Performance Gas Turbines," *MRS Bulletin*, p. 659-670, 2003.
- Onoda et al., "Preparation of Amorphous/Crystallloid Soft Magnetic Multilayer Ni—Co—B Alloy Films by Electrodeposition," *Journal of Magnetism and Magnetic Materials* 126(1-3):595-598, 1993.
- Parkin et al., "Oscillations in Exchange Coupling and Magnetoresistance in Metallic Superlattice Structures: Co/Ru, Co/Cr, and Fe/Cr," *Physical Review Letters* 64(19):2304-2307, 1990.
- Pilone et al., "Model of Multiple Metal Electrodeposition in Porous Electrodes," *Journal of the Electrochemical Society* 153(5):D85-D90, 2006.
- Podlaha et al. "Induced Codeposition: I. An Experimental Investigation of Ni—Mo Alloys," *J. Electrochem. Soc.* 143(3):885-892, 1996.
- Ross, "Electrodeposited Multilayer Thin Films," *Annual Review of Materials Science* 24:159-188, 1994.
- Rousseau et al., "Single-bath Electrodeposition of Chromium-Nickel Compositionally Modulated Multilayers (CMM) From a Trivalent Chromium Bath," *Plating and Surface Finishing*, p. 106-110, 1999.
- Saleh et al., "Effects of electroplating on the mechanical properties of stereolithography and laser sintered parts," *Rapid Prototyping Journal* 10(5)305-315, 2004.
- Sanders et al., "Mechanics of hollow sphere foams," *Materials Science and Engineering* A347:70-85, 2003.
- Sartwell et al., "Replacement of Chromium Electroplating on Gas Turbine Engine Components Using Thermal Spray Coatings," Report No. NPL/MR/6170-05-8890, Naval Research Laboratory, 2005. (207 pages).
- Schwartz, "Multiple-Layer Alloy Plating", ASM Handbook 5: Surface Engineering, p. 274-276, 1994.
- Sherik, "Synthesis, Structure and Properties of Electrodeposited Bulk Nanocrystalline Nickel", Master's Thesis, Queen's University, Ontario, Canada, 1993.
- Shishkovski, "Laser synthesis of functionally graded meso structures and bulk products," Fizmatlit, Moscow, Russia, pp. 30-38, 2009. (with English Abstract).
- Simunovich et al., "Electrochemically Layered Copper-Nickel Nanocomposites with Enhanced Hardness," *J. Electrochem. Soc.* 141(1):L10-L11, 1994.
- Sperling et al., "Correlation of stress state and nanohardness via heat treatment of nickel-aluminide multilayer thin films," *J. Mater. Res.* 19(11):3374-3381, 2004.
- Srivastava et al., "Corrosion resistance and microstructure of electrodeposited nickel-cobalt alloy coatings," *Surface & Coatings Technology* 207:3051-3060, 2006.
- Stephenson, Jr., "Development and Utilization of a High Strength Alloy for Electroforming," *Plating* 53(2): 183-192, 1966.
- Suresh, "Graded Materials for Resistance to Contact Deformation and Damage," *Science* 292:2447-2451, 2001.
- Switzer et al., "Electrodeposited Ceramic Superlattices," *Science* 247(4941):444-446, 1990.
- Tench et al., "Considerations in Electrodeposition of Compositionally Modulated Alloys," *J. Electrochem. Soc.* 737(10):3061-3066, 1990.
- Tench et al., "Enhanced Tensile Strength for Electrodeposited Nickel-Copper Multilayer Composites," *Metallurgical Transactions A* 15A):2039-2040, 1984.
- Thangaraj et al., "Corrosion behavior of composition modulated multilayer Zn—Co electrodeposits produced using a single-bath technique," *J. of Appl. Electrochem.* 39:339-345, 2009.
- Thangaraj et al., "Surface Modification by Compositionally Modulated Multilayered Zn—Fe Coatings," *Chinese Journal of Chemistry* 26:2285-2291, 2008.
- Tokarz et al., "Preparation, structural and mechanical properties of electrodeposited Co/Cu multilayers," *Phys. Stat. Soli* 5(11):3526-3529, 2008.
- Touchstone Research Laboratory, Ltd., Material Safety Data Sheet, CFOAM Carbon Foams, 2008. (4 pages).
- Vill et al., "Mechanical Properties of Tough Multiscalar Microlaminates," *Acta metall. mater.* 43(2):427-437, 1995.
- Voevodin et al., "Superhard, functionally gradient, nanolayered and nanocomposite diamond-like carbon coatings for wear protection," *Diamond and Related Materials* 7:463-467, 1998.
- Wearmouth et al., "Electroforming with Heat-Resistant, Sulfur-Harden Nickel," *Plating and Surface Finishing* 66(10):53-57, 1979.

(56)

**References Cited**

## OTHER PUBLICATIONS

- Weil et al., "Pulsed Electrodeposition of Layered Brass Structures," *Metallurgical Transactions A* 19A:A569-1573, 1988.
- Weil et al., "Properties of Composite Electrodeposits," U.S. Army Research Office, Final Report, Contract No. DAAL03-87-K-0047, U.S. Army Research Office, 21 pages, 1990.
- Wikipedia, "Gold," URL= <http://en.wikipedia.org/wiki/Gold>, version modified Nov. 3, 12 pages, 2008.
- Wikipedia, "Silver," URL= <http://en.wikipedia.org/wiki/Silver>, version modified Nov. 3, 12 pages, 2008.
- Wilcox, "Surface Modification With Compositionally Modulated Multilayer Coatings," *The Journal of Corrosion Science and Engineering* 6(Paper 52), 2004.
- Wu et al., "Preparation and characterization of superhard CN<sub>x</sub>/ZrN multilayers," *J. Vac. Sci. Technol. A* 15(3):946-950, 1997.
- Yahalom et al., "Formation of composition-modulated alloys by electrodeposition," *Journal of Materials Science* 22:499-503, 1987.
- Yang et al., "Effects of SiC sub-layer on mechanical properties of Tyranno-SA/SiC composites with multiple interlayers," *Ceramics International* 31:525-531, 2005.
- Yang et al., "Enhanced elastic modulus in composition-modulated gold-nickel and copper-palladium foils," *Journal of Applied Physics* 48(3):876-879, 1977.
- Yogesha et al., "Optimization of deposition conditions for development of high corrosion resistant Zn—Fe multilayer coatings," *Journal of Materials Processing Technology* 211:1409-1415, 2011.
- Zabludovsky et al., "The Obtaining of Cobalt Multilayers by Programme-controlled Pulse Current," *Transactions of the Institute of Metal Finishing* 75(5):203-204, 1997.
- Paz et al., "Nano-Laminated Alloys for Improved Return on Oilfield Assets," Society of Petroleum Engineers, 2016 (14 pages).
- Dulal et al., "Characterisation of Co—Ni(Cu)/Cu multilayers deposited from a citrate electrolyte in a flow channel cell," *Electrochimica Acta* 49:2041-2049, 2004.
- Kalantary et al., "The Production of Compositionally Modulated Alloys by Simulated High Speed Electrodeposition From a Single Solution," *Electrochimica Acta* 40(11):1609-1616, 1995.
- Nabiyouni et al., "Growth, characterization and magnetoresistive study of electrodeposited Ni/Cu and Co—Ni/Cu multilayers," *Journal of Crystal Growth* 275:e1259-e1262, 2005.

\* cited by examiner



FIG. 3A



FIG. 3B



FIG. 2A



FIG. 2B



FIG. 1A



FIG. 1B



FIG. 6A



FIG. 6B



FIG. 5A



FIG. 5B



FIG. 4A



FIG. 4B



FIG. 7A



FIG. 8A



FIG. 7B



FIG. 8B



FIG. 11A



FIG. 11B



FIG. 10A



FIG. 10B



FIG. 9A



FIG. 9B



**FIG. 12A**



**FIG. 13A**



**FIG. 12B**



**FIG. 13B**



FIG. 14



FIG. 15









FIG. 19

## 1

**METHOD AND APPARATUS FOR  
CONTINUOUSLY APPLYING  
NANOLAMINATE METAL COATINGS**

**CROSS-REFERENCE TO RELATED  
APPLICATIONS**

This application claims the benefit of U.S. Provisional Patent Application No. 62/052,345, filed Sep. 18, 2014, which application is incorporated herein by reference in its entirety. In addition the disclosures of U.S. Provisional Application No. 61/802,102, filed Mar. 15, 2013, and International Patent Application No. PCT/US2014/31101, filed Mar. 18, 2014, are incorporated by reference herein in their entirety.

**BACKGROUND**

Nanolaminate materials have become widely studied over the past several decades. As a result some desirable advanced performance characteristics of those materials have been discovered and their potential application in numerous fields recognized. While the potential application of nanolaminated materials in numerous areas, including civil infrastructure, automotive, aerospace, electronics, and other areas, has been recognized, the materials are on the whole not available in substantial quantities due to the lack of a continuous process for their production.

**SUMMARY**

Described herein are apparatus and methods for the continuous application of nanolaminated materials by electrodeposition.

In some embodiments, the method imparts a stable mechanical and chemical finish to materials (e.g., steel) that is resistant to corrosion or that can receive a durable finish (e.g., paint powder coat, etc.).

**BRIEF DESCRIPTION OF THE DRAWINGS**

FIGS. 1A and 1B show a top and side view, respectively, of a plating cell according to various embodiments disclosed herein;

FIGS. 2A and 2B show a top and side view, respectively, of a triple rinse unit according to various embodiments disclosed herein;

FIGS. 3A and 3B show a top and side view, respectively, of a combined plating cell and triple rinse unit according to various embodiments described herein;

FIGS. 4A and 4B show a top and side view, respectively, of a quintuple rinse unit according to various embodiments disclosed herein;

FIGS. 5A and 5B show a top and side view, respectively, of a combined plating cell and double rinse unit according to various embodiments disclosed herein;

FIGS. 6A and 6B show a top and side view, respectively, of a combined immersion cell and quintuple rinse unit according to various embodiments disclosed herein;

FIGS. 7A and 7B show a top and side view, respectively, of a forced air dryer according to various embodiments disclosed herein;

FIGS. 8A and 8B show a top and side view, respectively, of a strip puller according to various embodiments described herein;

## 2

FIGS. 9A and 9B show a top and side view, respectively, of a storage tank according to various embodiments described herein;

FIGS. 10A and 10B show a top and side view, respectively, of a storage tank according to various embodiments described herein;

FIGS. 11A and 11B show a top and side view, respectively, of a storage tank according to various embodiments described herein;

FIGS. 12A and 12B show a top and side view, respectively, of a storage tank according to various embodiments described herein;

FIGS. 13A and 13B show a top and side view, respectively, of a storage tank according to various embodiments described herein;

FIG. 14 shows a piping and instrumentation configuration for a plating cell according to various embodiments described herein;

FIG. 15 shows a piping and instrumentation configuration for a triple countercurrent rinse unit according to various embodiments described herein;

FIG. 16 shows a piping and instrumentation configuration for an immersion cell according to various embodiments described herein;

FIG. 17 shows a piping and instrumentation configuration for a chromate coating cell according to various embodiments described herein;

FIGS. 18A and 18B show top and side views, respectively, of a continuous nanolaminate coating process line including 15 plating cells according to various embodiments described herein; and

FIG. 19 shows a continuous processing apparatus for the application of nanolaminated coatings configured for conductive materials that can be rolled.

**DETAILED DESCRIPTION**

**1.0 Definitions**

“Electrolyte” as used herein means an electrolyte bath, plating bath, or electroplating solution from which one or more metals may be electroplated.

“Workpiece” means an elongated conductive material or loop of conductive material.

“Nanolaminate” or “nanolaminated” as used herein refers to materials or coatings that comprise a series of layers less than 1 micron.

All compositions given as percentages are given as percent by weight unless stated otherwise.

**2.0 Electrodeposition Apparatus for Continuous Application of Nanolaminated Coatings**

**55 2.1 Exemplary Electrodeposition Apparatus**

FIGS. 1A-19 show various process units that may be used in various combinations to form a continuous electrodeposition process line capable of performing the continuous application of nanolaminate coatings on conductive materials.

A main component of the process line is the plating cell 100 shown in FIGS. 1A and 1B. The plating cell 100 is where the application of nanolaminate coatings on conductive materials is carried out, and generally includes an enclosure 110, a cathode brush assembly 120, an anode assembly 130. As shown in FIGS. 1A and 1B, the plating cell 100 includes two each of the cathode brush assembly 120

and anode assembly 130 in enclosure 110 such that two workpieces can be plated in parallel.

The enclosure 110 is generally a tank or vessel in which the other components of the plating cell 100 are located. The enclosure 110 is capable of containing electrolyte solution within the walls of the enclosure 110. Any suitable material can be used for the enclosure, including, for example, polypropylene. The dimensions of the enclosure are generally not limited. In some embodiments, the enclosure is approximately 3 feet long, 2 feet wide, and 1 foot, 2 inches tall.

The enclosure 110 includes one or more inlets 111 where electrolyte solution can be introduced into the enclosure 110. The flow of electrolyte solution into the enclosure 110 via the inlets 111 can be controlled via flow control valves 112. In some embodiments, the inlets are positioned within the anode assembly 130 so that the inlets 110 provide electrolyte solution into the anode assembly 130 positioned within the enclosure 110. The enclosure 110 can also include one or more drains 113 for allowing electrolyte solution to be drained from the enclosure 110. The enclosure 110 can be covered with a fold back lid 114 so that the interior of the enclosure 110 can be sealed off from the outside environment. The enclosure 110 can also include one or more ventilation slots 115 for safely venting gases from the interior of the enclosure 110.

As shown in FIG. 1A, the enclosure 110 further includes an inlet passage 116 and an outlet passage 117 at opposite ends of the enclosure 110. The inlet passage 116 and the outlet passage 117 are generally narrow vertical slits (e.g., 0.5 inches wide) in the enclosure 110 through which the workpiece passes into and out of the enclosure 110. In some embodiments, the passages 116, 117 do not extend the entire height of the enclosure 110. In some embodiments, the passages 116, 117 terminate approximately 3 inches above the bottom of the enclosure 110. An inlet passage 116 and an outlet passage 117 is provided for each line in the enclosure 110. For example, in the configuration shown in FIG. 1A, the enclosure 110 will include two inlet passages 116 and two outlet passages 117, one each for the parallel two process lines in the enclosure 110.

Although not shown in the remaining figures, similar inlet and outlet passages can be provided in all of the units described herein to allow for passage of the workpiece into and out of the individual units.

The cathode brush assembly 120 provides a manner for passing a current to the workpiece that will serve as the cathode in the plating cell 100. Accordingly, the cathode brush assembly 120 typically includes a structure that is connected to a power supply (not shown in FIGS. 1A and 1B) and is capable of passing a current to the workpiece as it passes against the cathode brush assembly 120. The cathode brush assembly can be made from any material suitable for receiving a voltage and conductively passing a current to the workpiece.

In some embodiments, the cathode brush assembly 120 includes an arm 121 extending from the cathode brush assembly 120. The arm 121 extending from the cathode brush assembly 120 can terminate at a vertically oriented rod 122a. A second vertical rod 122b may be spaced apart from the vertically oriented rod 122a to thereby form a narrow passage between the vertically oriented rods 122a, 122b. The workpiece passes through this passage and contacts the vertically oriented rod 122a to thereby pass a current to the workpiece. In some embodiments, one or both of the rods 122a, 122b are flexible.

The anode assembly 130 is an open vessel or tank located within the larger enclosure 110. The anode assembly 130 may include one or more vertical pillars 131 positioned throughout the anode assembly 130. In some embodiments, such as shown in FIG. 1A, the pillars 131 form two rows. The workpiece travels between the two rows of pillars 131, which are used as safety guards against the workpiece contacting the anode 132 located between the pillars 131 and the side walls of the anode assembly. In some embodiments, the vertical pillars 131 are perforated riser tubes.

The anode 132 in the anode assembly 130 may be made of any material suitable for use in electrodeposition of nanolaminate layers on a conductive material. The anode is connected to the same power supply (not shown in FIGS. 1A and 1B) as the corresponding cathode brush assembly 120 to thereby provide for the flow of electrons through the electrolyte solution and formation of nanolaminate layers on the workpiece. Electrolyte solution is contained within the anode assembly 130, and as a result, the plating of material on the workpiece passing through the anode assembly 130 takes place in the anode assembly 130.

The anode (which serves as an anode except during reverse pulses) may be inert or may be active, in which case the anode will contain the metal species that is to be deposited and will dissolve into solution during operation.

In some embodiments, the distance between the workpiece travelling through the plating cell 100 and the anode 132 may be adjusted in order to adjust various characteristics of the nanolaminate layers being deposited on the workpiece, such as the thickness of the nanolaminate layers. In some embodiments, the anode 132 is adjustable and may be positioned closer to the side walls of the anode assembly (in order to create a greater distance between the workpiece and the anode) or closer to the pillars (in order to decrease the distance between the workpiece and the anode). In some embodiments, the location of the workpiece as it travels through the anode assembly can be adjusted in order to move it closer or further away from a specific side wall of the anode assembly. In such embodiments, moving the workpiece so that it does not travel along a center line of the anode assembly (and is therefore not equidistant between the anodes at either side wall of the anode assembly) can result in different nanolaminate coatings depositing on either side of the workpiece (e.g., nanolaminate layers of differing thicknesses).

As shown in FIG. 1A, the anode assembly 130 further includes an inlet passage 133 and an outlet passage 134 at opposite ends of the anode assembly 130. The inlet passage 133 and the outlet passage 134 are generally narrow vertical slits (e.g., 0.25 inches wide) in the anode assembly 130 through which the workpiece passes into and out of the anode assembly 130.

Although not shown in the remaining figures, similar inlet and outlet passages can be provided in any of the vessels disposed within larger units as described herein to allow for passage of the workpiece into and out of the vessels.

While not shown in FIGS. 1A and 1B, the plating cell, and more specifically, the anode assembly, may also include a mechanism for agitating the electrolyte solution. Mixing of electrolyte in the plating cell may be provided by solution circulation, a mechanical mixer, ultrasonic agitators, and/or any other manner of agitating a solution known to those of ordinary skill in the art. While bulk mixing can be provided by a mixer, which can be controlled or configured to operate at variable speeds during the electrodeposition process, the plating cell may optionally include one or more ultrasonic agitators. The ultrasonic agitators of the apparatus may be

configured to operate independently in a continuous or in a non-continuous fashion (e.g., in a pulsed fashion). In one embodiment, the ultrasonic agitators may operate at about 17,000 to 23,000 Hz. In another embodiment, they may operate at about 20,000 Hz.

With reference to FIGS. 2A and 2B, a rinse unit 200 is shown wherein electrolyte and/or other process solutions may be rinsed off the workpiece. The rinse unit 200 shown in FIGS. 2A and 2B is a triple rinse unit containing three rinse stages. The rinse unit 200 can include any suitable number of stages. For example, FIGS. 4A and 4B show a quintuple rinse unit 400 including five rinse stages, while FIGS. 5A and 5B show a double rinse unit 500 paired with a plating cell 100. The depth and height of the rinse unit will typically be the same as the plating cell (e.g., 2 feet wide, 1 foot, 2 inches deep), while the length of the rinse unit will depend on the number of stages. In some embodiments, the triple rinse unit shown in FIGS. 2A and 2B is 1 foot long, the quintuple rinse shown FIGS. 4A and 4B is 1 foot, 6 and  $\frac{5}{8}$  inches long, and the double rinse unit shown in FIGS. 5A and 5B is 8 and  $\frac{3}{4}$  inches long.

The rinse unit 200 generally includes an enclosure 210. The enclosure 210 is a closed tank or vessel through which the workpiece may pass. The enclosure 210 may be made from any suitable material, and in some embodiments, is made from polypropylene. The enclosure may include a lid 211 and an exhaust strip 212 for safely venting gas and vapor from the rinse unit 200. The enclosure 210 may also include inlet and outlet passages (not shown) located at either end of the enclosure to allow for the passage of the workpiece into and out of the enclosure 210. As with the inlet passages described above with respect to the enclosure 110 of the plating cell, the passages are generally narrow, vertical slits.

The rinse unit 200 further includes one or more spreader pipes 220 for each stage of the rinse unit 200. As shown in FIGS. 2A and 2B, each stage of the rinse unit 200 includes two spreader pipes 220. Rinse solution (e.g., water) is dispensed from the spreader pipes 220 to rinse process solution and/or other materials from the workpiece passing through the rinse unit 200. In some embodiments, the spreader pipe 220 is flexible tubing to allow for various positioning of the spreader pipe within the rinse unit 200.

Each spreader pipe 220 can be associated with a rinse inlet 221 that provides rinse solution into the rinse unit 200 via the spreader pipe 220. Each rinse inlet 221 may be controlled by a flow control valve 222. The rinse unit 200 may also include one or more drains 230 to allow for the draining of rinse solution and process solution from the rinse unit 200.

As shown in FIGS. 2A and 2B, the rinse unit may also include a cathode brush assembly 120. The cathode brush assembly is similar or identical to the cathode brush assembly 120 located in the plating cell 100 and described in greater detail above. The cathode brush assembly 120 serves as a guide to help guide the workpiece through the rinse unit. The cathode brush assembly 120 also provides a means to continue to charge the workpiece as it travels down the process line.

FIGS. 3A and 3B show a plating cell 100 and rinse unit 200 combined together to form a part of the overall process line for electrodeposition of nanolaminated material. In this configuration, the outlet passage 117 of the enclosure 110 of the plating cell is aligned with the inlet passage of the enclosure 210 of the rinse unit 200 so that the workpiece can move from the plating cell 100 into the rinse unit 200. In some embodiments, a saddle or seal (not shown) can be used to hold together the plating cell 100 and the rinse unit 200

and prevent leakage between the units. Similar saddles or seals can be used to join together any two units described herein in order to e.g., prevent leakage of process fluid out of the units and/or into an adjoining unit.

5 With reference now to FIGS. 6A and 6B, an immersion unit 600 combined with a rinse unit 200 (quintuple rinse) is shown. The immersion unit 600 can be used to carry out, for example, acid activation on the workpiece after the plating steps have been carried out. The immersion unit 600 generally includes an enclosure 610 and an immersion vessel 620 positioned within the enclosure 610.

The enclosure 610 is generally a tank or vessel suitable for containing the process solutions used in the acid activation step. The enclosure 610 can be made from any material suitable for containing the process solution used in an acid activation process. In some embodiments, the enclosure 610 includes one or more drains 611 for draining process solution out of the enclosure 610. The enclosure 610 may also include inlet and outlet passages which allow the workpiece to pass into and out of the enclosure 610. As described above with respect to, for example, the plating cell, the inlet and outlet passages may be narrow vertical gaps.

The immersion vessel 620 is a tank or vessel into which the process solution for acid activation is flowed. In some embodiments, the immersion vessel 620 includes a perforated plate floor through which process solution flows in order to fill the immersion vessel 620. Process solution may be introduced into the immersion vessel 620 via inlet 621.

15 30 Flow of process solution into the immersion vessel 620 via inlet 621 can be controlled by flow control valve 622. The immersion vessel 620 may also include one or more guide rollers 623 around which the workpiece winds in order to increase the amount of time the workpiece remains in the immersion vessel 620. The immersion vessel 620 may include an inlet passage and an outlet passage at opposite ends of the immersion vessel so that the workpiece can pass into and out of the immersion vessel. The inlet and outlet 35 40 passages are typically narrow vertical gaps. With reference to FIGS. 7A and 7B, a forced air dryer 700 suitable for use in the process line is shown. The forced air dryer 700 may be any suitable type of forced air dryer capable of drying the workpiece as it passes through the forced air dryer. As shown in FIGS. 7A and 7B, the forced air dryer 700 may be configured to include a narrow passage 710 through which the workpiece can pass. The narrow passage may be formed by insulated blocks 711. The forced air dryer 700 may be contained within an enclosure 720, such as the tank of a

50 vessel, that includes a lid 721. In some embodiments, hot air is introduced into the forced air dryer 700 from one or more inlets located under the forced air dryer 700. The dimensions of the forced air dryer are generally not limited. In some embodiments, the forced air dryer has the same height and width as the other units of the process line (e.g., 2 feet wide, 1 foot, 2 inches tall), while the length is 2 feet long.

55 FIGS. 8A and 8B show a strip puller 800 which can be used to pull the workpiece through the process line. The strip puller may include a plurality of rollers 810 which work to pull the workpiece through the process line. Any suitable number of rollers 810 can be used. In some embodiments, one of the rollers 810 can be a collection roller around which the processed workpiece is wound for storage. The rollers 810 can be positioned on top of a table 820 as shown in FIGS. 8A and 8B. As also shown in FIGS. 8A and 8B, the strip puller 800 can include a cathode brush assembly 120 for guiding the workpiece towards the rollers 810 and

applying a current to the workpiece. The strip puller 800 can be used to adjust the speed at which the workpiece is pulled through the process line.

FIGS. 9A, 9B, 10A, 10B, 11A, 11B, 12A, 12B, 13A, and 13B illustrate top and side views of various holding tanks suitable for use in the process line disclosed herein. The tanks are capable of holding a variety of process solutions, and will generally be made of various materials suitable for containing whatever type of process solution is to be held within the tank. Each tank may optionally include a cover where necessary. In some embodiments, the tanks may include partitions, such as shown in FIG. 10A.

FIG. 14 shows an exemplary piping and instrumentation configuration for a plating cell 100. The plating cell 100 is similar or identical to the plating cell shown in FIGS. 1A and 1B, including an enclosure 110, a cathode brush assembly 120, and an anode assembly 130 having an anode 132. The configuration includes a power supply 1410 and a holding tank 1420.

The holding tank 1420 is used to hold a supply of electrolyte solution. The holding tank 1420 further includes a pump 1421 and an input line 1422. The pump 1421 is used to pump electrolyte solution to the anode assembly 130 via line 1422. Line 1422 can be split one or more times so that a supply of electrolyte solution is provided to each inlet 111 (e.g., as in the case of the two inlets 111 shown in FIG. 14). The flow of the electrolyte solution from the holding tank 1420 into the anode assembly 130 can be controlled via the flow control valves 112. As shown in FIG. 14, the input line 1422 can also include various flow meters, pressure meters, and valves as desired. An outlet line 1423 can also be provided in order to return electrolyte solution back to the holding tank 1420. The outlet line 1423 fluidly connects the drains 113 in the enclosure 110 to the holding tank 1420.

The power supply 1410 is connected to each of the cathode brush assemblies 120 and anodes 132 located in the plating cell 100. A line 1411 connects a negative terminal of the power supply to the cathode brush assembly 120. A line 1412 connects a positive terminal to the anode 132.

FIG. 15 shows an exemplary piping and instrumentation configuration for a three stage rinsing unit 200. The rinsing unit 200 can be similar or identical to the rinse unit 200 shown in FIGS. 2A and 2B. The configuration includes a holding tank 1510 that includes two partitions 1511 to provide three separate holding areas within the holding tank 1510. A pump 1520 is provided in each area so that the process solution in each area can be pumped to the rinse unit. In some embodiments, the rinse unit 200 uses three separate process solutions, thus making the configuration shown in FIG. 15 well adapted for the three stage rinse unit 200. A line 1512 connects each area to an inlet 221 in the rinse unit 200. Each inlet 221 is associated with a spreader pipe 220. The line 1512 can be split in order to provide process solution to each inlet 221 within a stage of the rinse unit 200, and each line 1512 can include a flow control valve 222 in order to control the flow of rinse solution into the rinse unit 200. As shown in FIG. 15, the input lines 1511 can also include various flow meters, pressure meters, and valves as desired.

Outlet lines 1513 can also be provided to allow for the return of process solution back to the holding tank 1510. The outlet lines 1513 are in fluid communication with the drains 230 of the rinse unit.

With reference to FIG. 16, an exemplary piping and instrumentation configuration for an immersion unit 600 and a five stage rinsing unit 200 is shown. The immersion unit 600 and five stage rinsing unit 200 are similar or identical to those shown in FIGS. 6A and 6B. The configuration includes

two holding tanks 1610 and 1620. Holding tank 1610 holds process fluid for use in the immersion unit 600 and holding tank 1620 holds process fluid for the five stage rinse unit 200.

- 5 Holding tank 1610 includes a pump 1611 for pumping process fluid from the holding tank 1610 to the immersion unit 600. An inlet line 1612 extends between the pump 1611 and the inlet 621 in the immersion vessel 620. The line 1612 may be split into two more lines to feed multiple inlets 621. 10 As shown in FIG. 16, the line 1612 splits once so that two lines can fluidly connect with the inlet 621 in each of the two immersion vessels 620. The line 1612 can further include flow control valves 622 to control the flow of process fluid into the immersion vessels 620. The line 1612 can include various flow meters, pressure meters, and valves as desired. 15

An outlet line 1613 can also be provided to allow for the return of process solution back to the holding tank 1610. The outlet line 1613 is in fluid communication with the drain 611 of the enclosure 610.

- 20 Holding tank 1620 is similar to holding tank 1510 shown in FIG. 15. The holding tank includes two partitions 1621 to separate the holding tank 1620 into three separate holding areas. Each area includes a pump 1622 used for pumping process fluid from the holding tank to a stage of the rinse unit 200. Each pump 1622 is in fluid communication with an inlet line 1623 that terminates at the inlets 221 of the rinse unit 200. Each line 1623 can be split to service both different inlets 221 within a single stage and inlets in different stages of the rinse unit 200. For example, as shown in FIG. 15, an inlet line 1623 splits into four different lines so that two inlets 221 in one rinse stage and two inlets 221 in another, adjacent stage can be supplied by the one line 1623. Each line servicing an inlet 221 can include a flow control valve 222 for controlling the flow of process solution to the inlet. 25 30 35 Each line 1623 can include various flow meters, pressure meters, and valves as desired.

- Outlet lines 1624 can also be provided to allow for the return of process solution back to the holding tank 1620. The outlet line 1624 is in fluid communication with the drain 230 40 of the rinse unit 200. Where two or more stages are supplied with the same process solution via inlet line 1623, the outlet lines 1624 are arranged so that the drained process solution from adjacent stages using the same process solution are returned to the appropriate partitioned area of the holding tank 1620.

- FIG. 17 shows an exemplary piping and instrumentation configuration for a pH control system suitable for use in controlling the pH of the electrolyte solution used in a plating cell. The piping and instrumentation used to deliver electrolyte solution from the tank 1420 to the plating cell is similar or identical to the piping and instrumentation shown in FIG. 14. The tank 1420 further includes tank 1710 filled with process solution suitable for adjusting the pH of the electrolyte solution as needed. An inlet line 1720 is provided 50 from the tank 1710 to the tank 1420 so that process solution for adjusting the pH of the electrolyte solution can be delivered to the tank 1420 as needed. Instrumentation 1730 used to monitor the pH of the electrolyte solution is provided in the tank 1420. This instrumentation 1730 is capable of sending readings to control system 1740, which receives the pH readings and analyzes the information to determine if pH control is required. Where pH control is required, the control system 1740 sends a signal to instrumentation 1750 associated with tank 1710. This information is received and 55 processed by instrumentation 1750, with the result being a desired amount of pH control process solution being sent to the tank 1420.

In some embodiments, the tank 1420 may further include a mixer 1760 for mixing pH control process solution introduced into the tank with the electrolyte solution. In some embodiments, the mixing blade of the mixer 1760 may be located proximate the location where pH control process solution is introduced into the tank 1420.

FIGS. 18A and 18B illustrate an embodiment of a process line wherein a combination of various units disclosed herein are combined to carry out the electrodeposition of nanolaminate layers on a workpiece. In the process line shown in FIGS. 18A and 18B, the workpiece enters the process line on the left and exits the process on the right.

The process line may begin with one or more pre-processing units which aim to put the workpiece in better condition for the electrodeposition process. In some embodiments, the first unit in the process line 1800 is an alkaline cleaner unit 1810. The alkaline cleaner unit 1810 is similar to the plating cell shown in FIGS. 1A and 1B. The alkaline unit 1810 does not include a cathode brush assembly or anode. Instead, the anode assembly is filled with the alkaline cleaner and the workpiece is passed through the anode assembly to carry out a cleaning step.

Next, the process line includes an electro-cleaner unit 1820. The electro-cleaner unit 1820 is similar to the plating cell shown in FIGS. 1A and 1B. In this case and as shown in FIGS. 18A and 18B, the electro-cleaner unit 1820 includes the cathode brush assembly and the anode in the anode assembly so that electropolishing can be carried out on the workpiece to remove undesired material from the workpiece surface (e.g., material that may inhibit subsequent electrodeposition). Accordingly, a power source is provided for the electro-cleaner unit 1820 so that the workpiece (via the cathode brush assembly) and anode can be appropriately charged.

Following the electro-cleaner unit 1820, a rinse unit 1830 is provided. As shown in FIGS. 18A and 18B, the rinse unit 1830 includes three stages, although fewer or more stages can be used. Any rinse solution suitable for removing process solution used in the alkaline cleaner unit 1810 and the electro-cleaner unit 1820 can be used in the rinse unit 1830. As also shown in FIGS. 18A and 18B, the rinse unit 1830 may include a cathode brush assembly to help guide the workpiece through the rinse unit 1830 and provide a current to the workpiece as necessary. Accordingly, a power source may be provided for supplying a voltage to the cathode brush assembly in the rinse unit 1830.

Following the rinse unit 1830, a series of three acid activator units 1840 are provided. Three acid activator units 1840 are shown, but fewer or more acid activator units may be used as necessary. The acid activator units 1840 are similar to the alkaline cleaner unit 1810 in that the unit resembles the plating cell shown in FIGS. 1A and 1B, but with the anode and cathode brush assembly removed. The workpiece passes through the anode assembly in each acid activator 1840, which is filled with the process solution used for acid activation. Any material that is suitable for acid activation of the workpiece can be used in the acid activator cells 1840.

Following the acid activator units 1840, another rinse unit 1850 is provided. As shown in FIGS. 18A and 18B, the rinse unit 1850 includes three stages, although fewer or more stages can be used. Any rinse solution suitable for removing process solution used in the acid activation units 1840 can be used in the rinse unit 1850. As also shown in FIGS. 18A and 18B, the rinse unit 1850 may include a cathode brush assembly to help guide the workpiece through the rinse unit 1850 and provide a current to the workpiece as necessary.

Accordingly, a power source may be provided for supplying a voltage to the cathode brush assembly in the rinse unit 1850.

Following the rinse unit 1850, the workpiece passes through a plurality of plating cells 1860. As shown in FIGS. 18A and 18B, the process line includes 15 sequential plating cells through which the workpiece passes, although fewer or more plating cells can be used. Each plating cell is similar or identical to the plating cell shown in FIGS. 1A and 1B. 10 Significantly, each plating cell 1860 may be operated independent of the other plating cells 1860. Each plating cell may include its own power source which may be operated using different parameters than in other plating cells 1860 included in the process line 1800. Each plating cell may 15 include a different electrolyte solution. Each plating cell may use a different distance between the anode and the workpiece. Any other variable process parameter in the plating cell may be adjusted from one plating cell to another. In this manner, the process line may be used to carry out a variety 20 of different coating procedures, including depositing coatings of different materials and thicknesses on the workpiece.

The various power supplies used for the plating cells may control the current density in a variety of ways including applying two or more, three or more or four or more different average current densities to the workpiece as it moves 25 through the plating cell. In one embodiment, the power supply can control the current density in a time varying manner that includes applying an offset current, so that the workpiece remains cathodic when it is moved through the 30 plating cell and the electrode remains anodic even though the potential between the workpiece and the electrode varies. In another embodiment, the power supply varies the current density in a time varying manner which comprises varying one or more of: the maximum current, baseline current, 35 minimum current, frequency, pulse current modulation and reverse pulse current modulation.

Following the plating cells 1860, the process line 1800 may include a rinse unit 1870. The rinse unit 1870 shown in FIGS. 18A and 18B includes five stages (although fewer or 40 more stages can be used). The rinse unit 1870 may be similar or identical to the rinse unit shown in FIGS. 4A, 4B, and 16. The rinse unit 1870 may be configured to deliver one or more different process solutions that are suitable for rinsing the workpiece of the process solutions use in the plating cells. In some embodiments, the first stage of the rinse unit provides a first rinse solution, the second and third stages 45 provide a second rinse solution, and the fourth and fifth stages provide a third rinse solution. The rinse unit 1870 may also include a cathode brush assembly.

Following the rinse unit 1870, the process line 1800 may include various post processing units. In some embodiments, the rinse unit 1870 is followed by an acid activation unit 1880. The acid activation unit may be similar or identical to the immersion unit 600 shown in FIGS. 6A, 6B, 55 and 16. The acid activation unit 1880 includes an immersion vessel which is filled with process solution for carrying out acid activation. Any material suitable for carrying out acid activation on the work piece can be used. The workpiece passes through the immersion vessel, which prepares the 60 workpiece for subsequent post processing steps.

Following the acid activation unit 1880, the process line 1800 may include a chromate coating unit 1890. The chromate coating unit 1890 may be similar to the acid activators 1840 used in the preprocessing portion of the process line 1800. The chromate coating unit 1890 is therefore similar to the plating cell shown in FIGS. 1A and 1B, but without the anode or cathode brush assembly. The anode assembly is

## 11

filled with process solution for carrying out a chromate coating step, and the workpiece is passed through the anode assembly to expose the workpiece to the process solution.

Following the chromate coating unit 1890, the process line may include a rinse unit 1900. The rinse unit 1900 may be similar or identical to the rinse unit 1870, including the use of five stages and multiple rinse solutions. In the rinse unit 1900, the rinse solutions can be any rinse solutions suitable for rinsing the workpiece of process solutions used in the acid activation unit 1880 and the chromate coating unit 1890. The rinse unit 1900 may include a cathode brush assembly to guide the workpiece and to provide a voltage if necessary/desired.

Following the rinse unit 1900, the process line 1800 may include a forced air dryer 1910. The forced air dryer 1910 may be similar or identical to the forced air dryer shown in FIGS. 7A and 7B. The forced air dryer 1910 is used to dry the workpiece of the rinse solutions used in the rinse unit 1900.

The workpiece may be moved through the process line 1800 using a strip puller 1920 provided at the end of the process line 1800. The strip puller 1920 may be similar or identical to the strip puller shown in FIGS. 8A and 8B. The strip puller 1920 may serve as a rate control mechanism which can adjust the speed at which the workpiece is pulled through the process line.

## 2.2 Alternate Electrodeposition Apparatus

The continuous application of nanolaminate coatings on conductive materials can also be accomplished using an electrodeposition apparatus as shown in FIG. 19. The electrodeposition apparatus can comprise:

- at least a first electrodeposition cell 1 through which a conductive workpiece 2, which serves as an electrode in the cell, is moved at a rate;
- a rate control mechanism that controls the rate the workpiece is moved through the electrodeposition cell;
- an optional mixer for agitating electrolyte during the electrodeposition process (shown schematically in FIG. 19 as item 3);
- a counter electrode 4; and
- a power supply 8 controlling the current density applied to the workpiece in a time varying manner as it moves through the cell.

The rate control mechanism (throughput control mechanism) may be integral to one or more drive motors or the conveying system (e.g., rollers, wheels, pulleys, etc., of the apparatus), or housed in associated control equipment; accordingly, it is not shown in FIG. 1. Similarly the counter electrode may have a variety of configurations including, but not limited to, bars, plates, wires, baskets, rods, conformal anodes and the like, and accordingly is shown generically as a plate 4 at the bottom of the electrodeposition cell 1 in FIG. 19. The counter electrode, which functions as an anode except during reverse pulses, may be inert or may be active, in which case the anode will contain the metal species that is to be deposited and will dissolve into solution during operation.

Power supply 8 may control the current density in a variety of ways including applying two or more, three or more or four or more different average current densities to the workpiece as it moves through the electrodeposition cell(s). In one embodiment the power supply can control the current density in a time varying manner that includes applying an offset current, so that the workpiece remains cathodic when it is moved through the electrodeposition cell and the electrode remains anodic even though the potential between the workpiece and the electrode varies. In another

## 12

embodiment the power supply varies the current density in a time varying manner which comprises varying one or more of: the maximum current, baseline current, minimum current, frequency, pulse current modulation and reverse pulse current modulation.

The workpiece may be introduced to the electrolyte by immersion in said electrolyte or by spray application of the electrolyte to the workpiece. The application of the electrolyte to the workpiece may be modulated. The rate by which the workpiece is moved through the electrolyte may also be modulated.

Mixing of electrolyte in the electrodeposition cell is provided by solution circulation, a mechanical mixer and/or ultrasonic agitators. While bulk mixing can be provided by the mixer 3, which can be controlled or configured to operate at variable speeds during the electrodeposition process, the apparatus may optionally include one or more ultrasonic agitators which are shown schematically as blocks 5 in the apparatus of FIG. 19. The ultrasonic agitators of the apparatus may be configured to operate independently in a continuous or in a non-continuous fashion (e.g., in a pulsed fashion). In one embodiment the ultrasonic agitators may operate at about 17,000 to 23,000 Hz. In another embodiment they may operate at about 20,000 Hz. Mixing of the electrolyte may also occur in a separate reservoir and the mixed electrolyte may contact the workpiece by immersion or by spray application. Instead of one or more salts of a metal to be electroplated, the electrolyte may comprise two or more, three or more or four or more different salts of electrodepositable metals.

The apparatus may include a location from which the workpiece material is supplied (e.g., a payoff reel) and a location where the coated workpiece is taken up (e.g., a take-up reel, which may be part of a strip puller for conveying a workpiece through the apparatus). Accordingly, the apparatus may comprise a first location 6, from which the workpiece is moved to the electrodeposition cell and/or a second location 7 for receiving the workpiece after it has moved through the electrodeposition cell. Location 6 and location 7 are shown as spindles with reels in FIG. 19, however, they may also consist of racks for storing lengths of materials, folding apparatus, and even enclosures with one or more small openings, from which a workpiece (e.g., a wire, cable, strip or ribbon) is withdrawn or into which a coated workpiece is inserted.

In one embodiment the first and/or second location comprises a spool or a spindle. In such an embodiment the apparatus may be configured to electrodeposit a nanolaminate coating on a continuum of connected parts, wire, rod, sheet or tube that can be wound on the spool or around the spindle.

The apparatus may further comprise an aqueous or a non-aqueous electrolyte. The electrolyte may comprise salts of two or more, three or more or four or more electrodepositable metals.

In addition to the above-mentioned components, the apparatus may comprise one or more locations for treatment of the workpiece prior or subsequent to electrodeposition. In one embodiment the apparatus further includes one or more locations, between the first location and the electrodeposition cell, where the workpiece is contacted with one or more of: a solvent, an acid, a base, an etchant, and/or a rinsing agent to remove the solvent, acid, base, or etchant. In another embodiment the apparatus further includes one or more locations between the electrodeposition cell and a second location, where the coated workpiece is subject to

one or more of: cleaning with solvent, cleaning with acid, cleaning with base, passivation treatments and rinsing.

### 3.0 Electrodeposition Process for the Continuous Application of Nanolaminated Coatings on Workpieces

The disclosure provided in this section is equally applicable to the apparatus and methods described in sections 2.1 and 2.2.

#### 3.1 Workpieces

Workpieces may take a variety of forms or shapes. Workpieces may be, for example, in the form of wire, rod, tube, or sheet stock (e.g., rolls or folded sheets). Workpieces may be metal or other conductive strip, sheet or wire. Workpieces may also comprise a series of discrete parts that may be, for example, affixed to a sheet or webbing (e.g., metal netting or flexible screen) so as to form a sheet-like assembly that can be introduced into the electrodeposition cell in the same manner as substantially flat sheets that are to be coated with a nanolaminated by electrodeposition. Workpieces which are a series of discrete parts connected to form a strip must be connected by a conductive connector.

Virtually any material may be used as a workpiece, provided it can be rendered conductive and is not negatively affected by the electrolyte. The materials that may be employed as workpieces include, but are not limited to, metal, conductive polymers (e.g., polymers comprising polyaniline or polypyrrole), or non-conductive polymers rendered conductive by inclusion of conductive materials (e.g., metal powders, carbon black, graphene, graphite, carbon nanotubes, carbon nanofibers, or graphite fibers) or electroless application of a metal coating.

#### 3.2 Continuous Electrodeposition of Nanolaminated Coatings

Nanolamine coatings may be continuously electrodeposited by a method comprising:

moving a workpiece through an apparatus comprising one or more electrodeposition cell(s) at a rate, where the electrodeposition cell(s) each comprise an electrode and an electrolyte comprising salts of one or more metals to be electrodeposited; and controlling the mixing rate and/or the current density applied to the workpiece in a time varying manner as the workpiece moves through the cell(s), thereby electrodepositing a nanolaminated coating.

By controlling the current density applied to the workpiece in a time varying manner, nanolaminated coatings having layers varying in elemental composition and/or the microstructure of the electrodeposited material can be prepared. In one set of embodiments, controlling the current density in a time varying manner comprises applying two or more, three or more or four or more different current densities to the workpiece as it moves through the electrodeposition cell(s). In another embodiment, controlling the current density in a time varying manner includes applying an offset current, so that the workpiece remains cathodic when it is moved through the electrodeposition cell(s) and the electrode remains anodic, even though the potential between the workpiece and the electrode varies in time to produce nanolamination. In another embodiment controlling the current density in a time varying manner comprises varying one or more of: the baseline current, pulse current modulation and reverse pulse current modulation.

Nanolaminated coatings may also be formed on the workpiece as it passes through the electrodeposition cell(s) by controlling the mixing rate in a time varying manner. In

one embodiment, controlling the mixing rate comprises agitating the electrolyte with a mixer (e.g., impeller or pump) at varying rates. In another embodiment, controlling the mixing rate comprises agitating the electrolyte by operating an ultrasonic agitator in a time varying manner (e.g., continuously, non-continuously, with a varying amplitude over time, or in a series of regular pulses of fixed amplitude). In another embodiment, controlling the mixing rate comprises pulsing a spray application of the electrolyte to the workpiece.

In another embodiment, the nanolamine coatings may be formed by varying both the current density and the mixing rate simultaneously or alternately in the same electrodeposition process.

15 Regardless of which parameters are varied to induce nanolaminations in the coating applied to the workpiece as it is moved through the electrodeposition cell(s), the rate at which the workpiece passes through the cell(s) represents another parameter that can be controlled. In one embodiment 20 rates that can be employed are in a range of about 1 to about 300 feet per minute. In other embodiments, the rates that can be employed are greater than about 1, 5, 10, 30, 50, 100, 150, 200, 250 or 300 feet per minute, or from about 1 to about 30 feet per minute, about 30 to about 100 feet per minute, about 25 100 to about 200 feet per minute, about 200 to about 300 feet per minute, or more than about 300 feet per minute. Faster rates will alter the time any portion of the workpiece being plated remains in the electrodeposition cell(s). Accordingly, the rate of mass transfer (rate of electrodeposition) that must 30 be achieved to deposit the same nanolamine coating thickness varies with the rate the workpiece is moved through the cell(s). In addition, where processes employ variations in current density to achieve nanolamination, the rate the variation in current density occurs must also be increased 35 with an increasing rate of workpiece movement through the electrodeposition cell(s).

In one embodiment, the electrodeposition process may further include a step of moving the workpiece from a first location to the electrodeposition cell or a group of electrodeposition cell(s) (e.g., two or more, three or more, four or more, or five or more electrodeposition cells). In another embodiment, the electrodeposition process may further include a step of moving the workpiece from the electrodeposition cell or a group of electrodeposition cells to a second location for receiving the workpiece after electrodeposition of the nanolamine coating. In such embodiments, the apparatus may have 1, 2, 3, 4, 5, 6, 7, 8, 9, 10, 11, 12, 13, 45 14, 15, 16, or more electrodeposition cells that may each have separate power supplies for conducting electrodeposition in their respective cell. As such, the method may further comprise both moving the workpiece from a first location to the electrodeposition cell(s) and moving the workpiece from the electrodeposition cell to the second location.

#### 3.3 Nanolamine and Fine Grain Coating and Electrolyte Compositions for their Electrodeposition

Continuous electrodeposition of nanolamine coatings can be conducted from either aqueous or non-aqueous electrolytes comprising salts of the metals to be electrodeposited.

60 In one embodiment, electrodepositing a nanolamine coating comprises the electrodeposition of a layered composition comprising one or more, two or more, three or more or four or more different elements independently selected from Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr, wherein each of said independently selected metals is present at greater than about 0.1, about 0.05, about 0.01,

about 0.005 or about 0.001% by weight. In one such embodiment, electrodepositing a nanolaminate coating comprises electrodeposition of a layered composition comprising two or more different elements independently selected from Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr, wherein each of said independently selected metals is present at greater than about 0.005 or about 0.001% by weight. In another such embodiment, electrodepositing a nanolaminate coating comprises the electrodeposition of layers comprising two or more different metals, where the two or more different metals comprise: Zn and Fe, Zn and Ni, Co and Ni, Ni and Fe, Ni and Cr, Ni and Al, Cu and Zn, Cu and Sn, or a composition comprising Al and Ni and Co (AlNiCo). In any of those embodiments the nanolaminate coating may comprise at least one portion consisting of a plurality of layers, wherein each of said layers has a thickness in a range selected independently from: about 5 nm to about 250 nm, from about 5 nm to about 25 nm, from about 10 nm to about 30 nm, from about 30 nm to about 60 nm, from about 40 nm to about 80 nm, from about 75 nm to about 100 nm, from about 100 nm to about 120 nm, from about 120 nm to about 140 nm, from about 140 nm to about 180 nm, from about 180 nm to about 200 nm, from about 200 nm to about 225 nm, from about 220 nm to about 250 nm, or from about 150 nm to about 250 nm.

In another embodiment, the electrodeposited nanolaminate coating compositions comprise a plurality of first layers and second layers that differ in structure or composition. The first layers and second layers may have discrete or diffuse interfaces at the boundary between the layers. In addition, the first and second layers may be arranged as alternating first and second layers.

In embodiments where the electrodeposited nanolaminate coatings comprise a plurality of alternating first layers and second layers, those layers may comprise two or more, three or more, four or more, six or more, eight or more, ten or more, twenty or more, forty or more, fifty or more, 100 or more, 200 or more, 500 or more, 1,000 or more, 1,500 or more, 2,000 or more, 3,000 or more, 5,000 or more or 8,000 or more alternating first and second layers independently selected for each multilayer coating.

In one embodiment each first layer and each second layer comprises, consists essentially of, or consists of two, three, four or more elements independently selected from: Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr. In another embodiment, each first layer and each second layer comprises, consists essentially of, or consists of two, three, four or more elements independently selected from: Ag, Al, Au, Co, Cr, Cu, Fe, Mg, Mn, Mo, Ni, P, Sb, Sn, Mn, Pb, Ta, Ti, W, V, and Zn. In another embodiment, each first layer and each second layer comprises, consists essentially of, or consists of two, three, four or more elements independently selected from: Al, Au, Co, Cr, Cu, Fe, Mg, Mn, Mo, Ni, P, Sn, Mn, Ti, W, V, and Zn.

In one embodiment each first layer comprises nickel in a range independently selected from about 1% to about 5%, about 5% to about 7%, about 7% to about 10%, about 10% to about 15%, about 15% to about 20%, about 20% to about 30%, about 30% to about 40%, about 40% to about 50%, about 50% to about 55%, about 55% to about 60%, about 60% to about 65%, about 65% to about 70%, about 70% to about 75%, about 75% to about 80%, about 80% to about 85%, about 85% to about 90%, about 90% to about 92%, about 92% to about 93%, about 93% to about 94%, about 94% to about 95%, about 95% to about 96%, about 96% to

about 97%, about 97% to about 98% or about 98% to about 99%. In such an embodiment, each second layer may comprise cobalt and/or chromium in a range independently selected from about 1% to about 35%, about 1% to about 3%, about 2% to about 5%, about 5% to about 10%, about 10% to about 15%, about 15% to about 20%, about 20% to about 25%, about 25% to about 30% or about 30% to about 35%.

In one embodiment each first layer comprises nickel in a range independently selected from about 1% to about 5%, about 5% to about 7%, about 7% to about 10%, about 10% to about 15%, about 15% to about 20%, about 20% to about 30%, about 30% to about 40%, about 40% to about 50%, about 50% to about 55%, about 55% to about 60%, about 60% to about 65%, about 65% to about 70%, about 70% to about 75%, about 75% to about 80%, about 80% to about 85%, about 85% to about 90%, about 90% to about 92%, about 92% to about 93%, about 93% to about 94%, about 94% to about 95%, about 95% to about 96%, about 96% to about 97%, about 97% to about 98% or about 98% to about 99%, and the balance of the layer comprises cobalt and/or chromium. In such an embodiment, each second layer may comprise cobalt and/or chromium in a range selected independently from about 1% to about 35%, about 1% to about 3%, about 2% to about 5%, about 5% to about 10%, about 10% to about 15%, about 15% to about 20%, about 20% to about 25%, about 25% to about 30% or about 30% to about 35%, and the balance of the layer comprises nickel. In such embodiments, first and second layers may additionally comprise aluminum.

In one embodiment each first layer comprises nickel in a range independently selected from about 1% to about 5%, about 5% to about 7%, about 7% to about 10%, about 10% to about 15%, about 15% to about 20%, about 20% to about 30%, about 30% to about 40%, about 40% to about 50%, about 50% to about 55%, about 55% to about 60%, about 60% to about 65%, about 65% to about 70%, about 70% to about 75%, about 75% to about 80%, about 80% to about 85%, about 85% to about 90%, about 90% to about 92%, about 92% to about 93%, about 93% to about 94%, about 94% to about 95%, about 95% to about 96%, about 96% to about 97%, about 97% to about 98% or about 98% to about 99%, and the balance of the layer comprises aluminum. In such an embodiment, each second layer may comprise aluminum in a range selected independently from about 1% to about 35%, about 1% to about 3%, about 2% to about 5%, about 5% to about 10%, about 10% to about 15%, about 15% to about 20%, about 20% to about 25%, about 25% to about 30% or about 30% to about 35%, and the balance of the layer comprises nickel.

In one embodiment each first layer comprises nickel in a range independently selected from about 1% to about 5%, about 5% to about 7%, about 7% to about 10%, about 10% to about 15%, about 15% to about 20%, about 20% to about 30%, about 30% to about 40%, about 40% to about 50%, about 50% to about 55%, about 55% to about 60%, about 60% to about 65%, about 65% to about 70%, about 70% to about 75%, about 75% to about 80%, about 80% to about 85%, about 85% to about 90%, about 90% to about 92%, about 92% to about 93%, about 93% to about 94%, about 94% to about 95%, about 95% to about 96%, about 96% to about 97%, about 97% to about 98% or about 98% to about 99%, and the balance of the layer comprises iron. In such an embodiment, each second layer may comprise iron in a range independently selected from about 1% to about 35%, about 1% to about 3%, about 2% to about 5%, about 5% to about 10%, about 10% to about 15%, about 15% to about 20%, about 20% to about 25%, about 25% to about 30% or about 30% to about 35%, and the balance of the layer comprises iron.

20%, about 20% to about 25%, about 25% to about 30% or about 30% to about 35%, and the balance of the layer comprises nickel.

In one embodiment each first layer comprises zinc in a range independently selected from about 1% to about 5%, about 5% to about 7%, about 7% to about 10%, about 10% to about 15%, about 15% to about 20%, about 20% to about 30%, about 30% to about 40%, about 40% to about 50%, about 50% to about 55%, about 55% to about 60%, about 60% to about 65%, about 65% to about 70%, about 70% to about 75%, about 75% to about 80%, about 80% to about 85%, about 85% to about 90%, about 90% to about 92%, about 92% to about 93%, about 93% to about 94%, about 94% to about 95%, about 95% to about 96%, about 96% to about 97%, about 97% to about 98%, about 98% to about 99%, about 99% to about 99.5%, about 99.2% to about 99.7%, or about 99.5% to about 99.99%, and the balance of the layer comprises iron. In such an embodiment, each second layer may comprise iron in a range independently selected from about 0.01% to about 35%, about 0.01% to about 0.5%, about 0.3% to about 0.8%, about 0.5% to about 1.0%, about 1% to about 3%, about 2% to about 5%, about 5% to about 10%, about 10% to about 15%, about 15% to about 20%, about 20% to about 25%, about 25% to about 30% or about 30% to about 35%, and the balance of the layer comprises zinc.

In any of the foregoing embodiments the first and/or second layers may each comprise one or more, two or more, three or more, or four or more elements selected independently for each first and second layer from the group consisting of Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr.

In one embodiment, electrodepositing a "fine-grained" or "ultrafine-grained" metal comprises electrodepositing a metal or metal alloy having an average grain size from 1 nm to 5,000 nm (e.g., 1-20, 1-100, 5-50, 5-100, 5-200, 10-100, 10-200, 20-200, 20-250, 20-500, 50-250, 50-500, 100-500, 200-1,000, 500-2,000, or 1,000-5,000 nm based on the measurement of grain size in micrographs). In such embodiments, the fine-grained metal or alloy may comprise one or more, two or more, three or more, or four or more elements selected independently from the group consisting of Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr. Fine-grained metals and alloys, including those comprising a high degree of twinning between metal grains, may remain ductile while having one or more properties including increased hardness, tensile strength, and corrosion resistance relative to electrodeposited metals or alloys of the same composition with a grain size from 5,000 to 20,000 nm or greater.

In one embodiment, the coefficient of thermal expansion of the nanolaminate coating layers and/or the fine grain coating layers is within 20% (less than 20%, 15%, 10%, 5%, or 2%) of the workpiece in the direction parallel to workpiece movement (i.e., in the plane of the workpiece and parallel to the direction of workpiece movement).

### 3.4 Pre- and Post-Electrodeposition Treatments

Prior to electrodeposition, or following electrodeposition, methods of continuously electrodepositing a nanolaminate coating may include further steps of pre-electrodeposition or post-electrodeposition treatment.

Accordingly, the apparatus described above may further comprise one or more locations between the first location and the electrodeposition cell(s), and the method may further comprise contacting the workpiece with one or more of:

a solvent, an acid, a base, an etchant, or a rinsing solution (e.g., water) to remove said solvent, acid, base, or etchant. In addition, the apparatus described above may further comprise one or more locations between the electrodeposition cell(s) and a second location, and the method may further comprise contacting the workpiece with one or more of: a solvent, an acid, a base, a passivation agent, or a rinse solution (e.g., water) to remove the solvent, acid, base or passivation agent.

### 4.0 Nanolaminated Articles Prepared by Continuous Electrodeposition

The disclosure provided in this section is equally applicable to the apparatus and methods described in sections 2.1 and 2.2

The process and apparatus described herein may be adapted for the preparation of articles comprising, consisting essentially of, or consisting of nanolaminated materials by the use of a workpiece to which the coating applied during electrodeposition does not adhere tightly. The article may be obtained after removal of the workpiece from the electrodeposition process by separating the coating from the workpiece. In addition, where the workpiece is not flat, 3-dimensional articles may be formed as reliefs on the contoured surface of the workpiece.

### 5.0 Certain Embodiments

1. An apparatus for electrodepositing a nanolaminate coating comprising:

at least a first electrodeposition cell and a second electrodeposition cell (e.g., two, three, four, five, six, seven, eight, nine, ten, eleven, twelve, thirteen, fourteen, fifteen, sixteen or more electrodeposition cells) through which a conductive workpiece is moved at a rate, each electrodeposition cell containing an electrode (e.g., an anode); and

a rate control mechanism that controls the rate the workpiece is moved through the electrodeposition cell(s); wherein each electrodeposition cell optionally comprises a mixer for agitating an electrolyte in its respective electrodeposition cell during the electrodeposition process;

wherein each electrodeposition cell optionally comprises a flow control unit for applying an electrolyte to the workpiece; and

wherein each electrodeposition cell has a power supply (e.g., a power supply for each cell or groups of cells comprising two, three, four, five, six, seven, eight, nine, ten, eleven, twelve, thirteen, fourteen or fifteen cells) controlling the current density and/or voltage applied to the workpiece in a time varying manner as it moves through each electrodeposition cell.

2. The apparatus of embodiment 1, wherein controlling the current density in a time varying manner comprises applying two or more, three or more or four or more different current densities to the workpiece as it moves through at least one electrodeposition cell (e.g., two or more, three or more, four or more, five or more, or each electrodeposition cell).

3. The apparatus of embodiment 2, wherein controlling the current density in a time varying manner comprises applying an offset current, so that the workpiece remains cathodic when it is moved through at least one electrodeposition cell (e.g., one or more, two or more, three or more, four or more, five or more, or each electrodeposition cell) and the electrode remains anodic.

4. The apparatus of any of embodiments 1 or 2, wherein the time varying manner comprises one or more of: varying the baseline current, pulse current modulation and reverse pulse current modulation.
5. The apparatus of any of the preceding embodiments, wherein one or more of the electrodeposition cells further comprises an ultrasonic agitator.
6. The apparatus of embodiment 5, wherein each ultrasonic agitator independently operates continuously or in a pulsed fashion.
7. The apparatus of any of the preceding embodiments, wherein at least one electrodeposition cell (e.g., one or more, two or more, three or more, four or more, five or more, or each electrodeposition cell) comprises a mixer that operates independently to variably mix an electrolyte placed in its respective electrodeposition cell(s).
8. The apparatus of any of the preceding embodiments, further comprising a first location, from which the workpiece is moved to the electrodeposition cells, and/or a second location, for receiving the workpiece after it has moved through one or more of the electrodeposition cells.
9. The apparatus of embodiment 8, wherein the first and/or second location comprises a spool or a spindle.
10. The apparatus of embodiment 9, wherein the workpiece is a wire, rod, sheet, chain, strand, or tube that can be wound on said spool or around said spindle.
11. The apparatus of any of the preceding embodiments, wherein any one or more of said electrodeposition cell(s) (e.g., one or more, two or more, three or more, four or more, five or more, or each electrodeposition cell) comprises (contains) an aqueous electrolyte.
12. The apparatus of any of embodiments 1-10, wherein any one or more of said electrodeposition cell(s) (e.g., one or more, two or more, three or more, four or more, five or more, or each electrodeposition cell) comprises (contains) a non-aqueous electrolyte.
13. The apparatus of any preceding embodiment, wherein each electrolyte comprises salts of two or more, three or more or four or more electrodepositable metals, which are selected independently for each electrolyte.
14. The apparatus of any of the preceding embodiments further comprising one or more locations between the first location and the electrodeposition cells, where the workpiece is contacted with one or more of: a solvent, an acid, a base, an etchant, and a rinsing agent to remove said solvent, acid, base, or etchant.
15. The apparatus of any of the preceding embodiments further comprising one or more locations between the electrodeposition cells and said second location, where the coated workpiece is subject to one or more of: cleaning with solvent, cleaning with acid, cleaning with base, passivation treatments, or rinsing.
16. A method of electrodepositing a nanolaminate coating comprising:

providing an apparatus comprising at least a first electrodeposition cell and a second electrodeposition cell (e.g., two, three, four, five, six, seven, eight, nine, ten, eleven, twelve, thirteen, fourteen, fifteen or more electrodeposition cells);

wherein each electrodeposition cell has a power supply (e.g., a power supply for each cell or groups of cells comprising two, three, four, five, six, seven, eight, nine, ten, eleven, twelve, thirteen, fourteen or fifteen cells) controlling the current density applied to the workpiece in a time varying manner as it moves through each electrodeposition cell;

- where each electrodeposition cell comprises an electrode and an electrolyte comprising salts of two or more, three or more, or four or more different electrodepositable metals selected independently for each electrolyte; and
- 5 moving a workpiece through at least the first electrodeposition cell and the second electrodeposition cell of the apparatus at a rate and independently controlling the mixing rate and/or the current density applied to the workpiece in a time varying manner as it moves through each electrodeposition cell, thereby electrodepositing a coating comprising nanolaminate coating layers and/or one or more (e.g., two or more, three or more, four or more, or five or more) fine-grained metal layers.
17. The method of embodiment 16, wherein controlling the current density in a time varying manner comprises applying two or more, three or more, or four or more different current densities to the workpiece as it moves through at least one electrodeposition cell (e.g., two or more, three or more, four or more, or five or more electrodeposition cells).
18. The method of embodiment 16 or 17, wherein controlling the current density in a time varying manner comprises applying an offset current, so that the workpiece remains cathodic when it is moved through at least one electrodeposition cell (e.g., two or more, three or more, four or more, or five or more electrodeposition cells) and the electrode remains anodic.
19. The method of embodiments 16 or 17, wherein the time varying manner comprises one or more of: varying the baseline current, pulse current modulation and reverse pulse current modulation.
20. The method of any of embodiments 16-19, wherein one or more electrodeposition cells comprises a mixer, wherein each mixer is independently operated at a single rate or at varying rates to agitate the electrolyte within its respective electrodeposition cell.
21. The method of any of embodiments 16-20, wherein one or more electrodeposition cells comprises an ultrasonic agitator, wherein each agitator is independently operated continuously or in a non-continuous fashion to control the mixing rate.
22. The method of any of embodiments 16-21, further comprising controlling the rate the workpiece is moved through the electrodeposition cells.
23. The method of any of embodiments 16-22, wherein the apparatus further comprises a first location, from which the workpiece is moved to the first electrodeposition cell and the second electrodeposition cell (e.g., the electrodeposition cells), and/or a second location for receiving the workpiece after it has moved through the first electrodeposition cell and the second electrodeposition cell (e.g., the electrodeposition cells), the method further comprising moving the workpiece from the first location to the first electrodeposition cell and the second electrodeposition cell and/or moving the workpiece from the first electrodeposition cell and the second electrodeposition cell to the second location.
24. The method of embodiment 23, wherein the apparatus further comprises one or more locations between the first location and the electrodeposition cell(s), and the method further comprises contacting the workpiece with one or more of: a solvent, an acid, a base, and an etchant, and rinsing to remove said solvent, acid, base, or etchant at one or more of the locations between the first location and the electrodeposition cell(s).
25. The method of embodiments 23 or 24, wherein the apparatus further comprises one or more locations between the electrodeposition cells and said second location, and the method further comprises contacting the workpiece with one

or more of: a solvent, an acid, a base, a passivation agent, and a rinsing agent to remove the solvent, acid, base and/or passivation agent at one or more locations between the electrodeposition cells and said second location.

26. The method of any of embodiments 16-25, wherein said workpiece is comprised of a metal, a conductive polymer or a non-conductive polymer rendered conductive by inclusion of conductive materials or electroless application of a metal.

27. The method of any of embodiments 16-26, wherein the workpiece is a wire, rod, sheet, chain, strand, or tube.

28. The method of any of embodiments 16-27, wherein the electrolytes is/are aqueous electrolyte(s) (e.g., one or more, two or more, or each electrolyte is an aqueous electrolyte).

29. The method of any of embodiments 16-27, wherein the electrolyte(s) is/are a non-aqueous electrolyte(s) (e.g., one or more, two or more, or each electrolyte is a non-aqueous electrolyte).

30. The method of any of embodiments 16-29, wherein electrodepositing a nanolaminate coating or fine grained metal comprises the electrodeposition of a composition comprising one or more, two or more, three or more or four or more different elements independently selected from Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr, wherein each of said independently selected metals is present at greater than 0.1, 0.05, 0.01, 0.005 or 0.001% by weight.

31. The method of any of embodiments 16-29, wherein electrodepositing a nanolaminate coating or fine grained metal comprises the electrodeposition of a composition comprising two or more different elements independently selected from Ag, Al, Au, Be, Co, Cr, Cu, Fe, Hg, In, Mg, Mn, Mo, Nb, Nd, Ni, P, Pd, Pt, Re, Rh, Sb, Sn, Pb, Ta, Ti, W, V, Zn and Zr, wherein each of said independently selected metals is present at greater than about 0.1, 0.05, 0.01, 0.005 or 0.001% by weight.

32. The method of embodiment 31, wherein said two or more different metals comprise: Zn and Fe, Zn and Ni, Co and Ni, Ni and Fe, Ni and Cr, Ni and Al, Cu and Zn, Cu and Sn, or a composition comprising Al and Ni and Co.

33. The method according to any of embodiments 16-32, wherein the nanolaminate coating comprises at least one portion consisting of a plurality of layers, wherein each of said layers has a thickness in a range selected independently from about 5 nm to about 250 nm, from about 5 nm to about 25 nm, from about 10 nm to about 30 nm, from about 30 nm to about 60 nm, from about 40 nm to about 80 nm, from about 75 nm to about 100 nm, from about 100 nm to about 120 nm, from about 120 nm to about 140 nm, from about 140 nm to about 180 nm, from about 180 nm to about 200 nm, from about 200 nm to about 225 nm, from about 220 nm to about 250 nm, or from about 150 nm to about 250 nm.

34. The method of any of embodiments 16-33, wherein the nanolaminate coating layers comprise a plurality of first layers and second layers that differ in structure or composition, and which may have discrete or diffuse interfaces between the first and second layers.

35. The method of embodiment 34, wherein the first and second layers are arranged as alternating first and second layers.

36. The method of embodiment 35, wherein said plurality of alternating first layers and second layers comprises two or more, three or more, four or more, six or more, eight or more, ten or more, twenty or more, forty or more, fifty or more, 100 or more, 200 or more, 500 or more, 1,000 or more, 1,500 or more, 2,000 or more, 4,000 or more, 6,000 or more,

or 8,000 or more alternating first and second layers independently selected for each multilayer coating.

37. The method of any of embodiments 34-36, wherein each first layer comprises nickel in a range independently selected from 1%-5%, 5%-7%, 7%-10%, 10%-15%, 15%-20%, 20%-30%, 30%-40%, 40%-50%, 50%-55%, 55%-60%, 60%-65%, 65%-70%, 70%-75%, 75%-80%, 80%-85%, 85%-90%, 90%-92%, 92%-93%, 93%-94%, 94%-95%, 95%-96%, 96%-97%, 97%-98% or 98%-99%.

10 38. The method of embodiment 37, wherein each second layer comprises cobalt and/or chromium in a range independently selected from 1%-35%, 1%-3%, 2%-5%, 5%-10%, 10%-15%, 15%-20%, 20%-25%, 25%-30% or 30%-35%.

15 39. The method of any of embodiments 34-36, wherein each first layer comprises nickel in a range independently selected from 1%-5%, 5%-7%, 7%-10%, 10%-15%, 15%-20%, 20%-30%, 30%-40%, 40%-50%, 50%-55%, 55%-60%, 60%-65%, 65%-70%, 70%-75%, 75%-80%, 80%-85%, 85%-90%, 90%-92%, 92%-93%, 93%-94%, 94%-95%, 95%-96%, 96%-97%, 97%-98% or 98%-99%, and the balance of the layer comprises, consists essentially of, or consists of cobalt and/or chromium.

20 40. The method of embodiment 39, wherein each second layer comprises cobalt and/or chromium in a range selected independently from 1%-35%, 1%-3%, 2%-5%, 5%-10%, 10%-15%, 15%-20%, 20%-25%, 25%-30% or 30%-35%, and the balance of the layer comprises, consists essentially of nickel.

25 41. The method of any of embodiments 34-36, wherein each first layer comprises nickel in a range independently selected from 1%-5%, 5%-7%, 7%-10%, 10%-15%, 15%-20%, 20%-30%, 30%-40%, 40%-50%, 50%-55%, 55%-60%, 60%-65%, 65%-70%, 70%-75%, 75%-80%, 80%-85%, 85%-90%, 90%-92%, 92%-93%, 93%-94%, 94%-95%, 95%-96%, 96%-97%, 97%-98% or 98%-99%, and the balance of the layer comprises, consists essentially of, or consists of iron.

30 42. The method of embodiment 41, wherein each second layer comprises iron in a range independently selected from 1%-35%, 1%-3%, 2%-5%, 5%-10%, 10%-15%, 15%-20%, 20%-25%, 25%-30% or 30%-35%, and the balance of the layer comprises, consists essentially of, or consists of nickel.

35 43. The method of any of embodiments 34-36, wherein each first layer comprises zinc in a range independently selected from 1%-5%, 5%-7%, 7%-10%, 10%-15%, 15%-20%, 20%-30%, 30%-40%, 40%-50%, 50%-55%, 55%-60%, 60%-65%, 65%-70%, 70%-75%, 75%-80%, 80%-85%, 85%-90%, 90%-92%, 92%-93%, 93%-94%, 94%-95%, 95%-96%, 96%-97%, 97%-98%, 98%-99%, 99%-99.5%, 99.2%-99.7%, or 99.5%-99.99%, and the balance of the layer comprises, consists essentially of, or consists of iron.

40 44. The method of embodiment 43, wherein each second layer comprises iron in a range independently selected from 0.01%-35%, 0.01%-0.5%, 0.3%-0.8%, 0.5%-1.0%, 1%-3%, 2%-5%, 5%-10%, 10%-15%, 15%-20%, 20%-25%, 25%-30% or 30%-35%, and the balance of the layer comprises, consists essentially of, or consists of zinc.

45 45. The method of any of embodiments 34-36, wherein one or more of said first and/or second layers comprises one or more, two or more, three or more or four or more elements selected independently for each first and second layer from the group consisting of Ag, Al, Au, C, Cr, Cu, Fe, Mg, Mn, Mo, Sb, Si, Sn, Pb, Ta, Ti, W, V, Zn and Zr.

50 46. A product produced by the method of any of embodiments 16-45.

The invention claimed is:

1. An apparatus for continuously electrodepositing a nanolaminate coating on a workpiece, comprising:
  - a. an electrodeposition cell including an anode assembly and a cathode assembly, the anode assembly including an anode having a first portion and a second portion that is spaced apart from the first portion and a plurality of pillars arranged in two rows with a first row adjacent to the first portion of the anode and a second row adjacent to the second portion of the anode and configured to guard against the workpiece contacting the anode located between the pillars and side walls of the anode assembly when the workpiece travels between the two rows of the pillars, wherein the pillars in each of the two rows are evenly spaced along a length of the anode; 15
  - b. a plurality of rollers around which the workpiece is wound, the plurality of rollers defining a path for passing the workpiece through the electrodeposition cell, the path causing the workpiece not to travel along a center line formed by the first portion and the second portion of the anode assembly, such that a first nanolaminate coating is electrodeposited onto a first surface of the workpiece and a second nanolaminate coating is electrodeposited onto a second surface of the workpiece as the workpiece moves through the electrodeposition cell, the first nanolaminate coating having a first thickness and the second nanolaminate coating having a second thickness that is different than the first thickness; 20
  - c. a rate control mechanism configured to control a rate at which the workpiece is moved through the electrodeposition cell; and
  - d. a power supply electrically connected to the anode assembly and configured to control a current density applied to the workpiece in a time varying manner as the workpiece moves through the electrodeposition cell, wherein the power supply is configured to apply two or more different current densities to the workpiece as it moves through the electrodeposition cell and to supply an offset current to the anode assembly such that the workpiece remains cathodic as the workpiece moves through the electrodeposition cell. 30
2. The apparatus of claim 1, wherein the electrodeposition cell further comprises an ultrasonic agitator.
3. The apparatus of claim 1, wherein the electrodeposition cell further comprises a mixer configured to mix an electrolyte in the electrodeposition cell.
4. The apparatus of claim 1, wherein the workpiece is a wire, rod, sheet, chain, strand, or tube configured to be wound at least partially around each of the plurality of rollers. 45
5. The apparatus of claim 1, further comprising a location upstream of the electrodeposition cell configured to contact the workpiece with one or more of: a solvent, an acid, a base, an etchant, and a rinsing agent to remove the solvent, acid, base, or etchant.
6. The apparatus of claim 1 further comprising a location downstream from the electrodeposition cell configured to contact the workpiece with one or more of: a solvent, an acid, a base, a passivation treatment, or rinsing agent. 60
7. The apparatus of claim 1 further comprising:
  - a. a strip puller configured to move the workpiece along the path, the strip puller including a cathode brush assembly configured to apply a current to the workpiece. 65

8. The apparatus of claim 1, wherein the power supply is configured to apply three or more different current densities to the workpiece as it moves through the electrodeposition cell.
9. An apparatus for continuously electrodepositing a nanolaminate coating on a workpiece, comprising:
  - a. an electrodeposition cell comprising:
    - a. an anode assembly, the anode assembly comprising an anode including a first portion and a second portion spaced apart from the first portion;
    - b. a cathode assembly; and
    - c. a plurality of pillars positioned throughout a length of the anode assembly and arranged into a first row and a second row spaced apart from the first row, wherein the pillars in the first row are spaced from the first portion of the anode by a first distance and the pillars in the second row are spaced from the second portion of the anode assembly by a second distance greater than the first distance;
    - d. a plurality of rollers that define a path along which the workpiece passes through the electrodeposition cell, the path being spaced apart from each of the plurality of pillars, the plurality of pillars being guards against the workpiece contacting the anode assembly as the workpiece moves through the electrodeposition cell; and
  - b. a power supply electrically connected to the electrodeposition cell, the power supply configured to apply an offset current having two or more different current densities to the workpiece in a time varying manner as the workpiece moves through the electrodeposition cell.
10. The apparatus of claim 9 wherein the pillars in the plurality of pillars have the same dimension.
11. The apparatus of claim 9 wherein the first portion of the anode is configured to be adjustable so that the first position of the anode between a first side wall of the anode assembly and the first row of the plurality of pillars is positioned either closer to the first side wall of the anode assembly or closer to the first row of the plurality of pillars to vary a distance between the first portion of the anode and the workpiece.
12. The apparatus of claim 9 wherein the plurality of rollers are configured to be adjustable to vary the path and adjust a distance between the workpiece and respective first and second portions of the anode.
13. The apparatus of claim 9 wherein the path is a first distance from the first portion of the anode and a second distance from the second portion of the anode, the second distance being different than the first distance.
14. The apparatus of claim 9 further comprising:
  - a. a strip puller configured to move the workpiece along the plurality of rollers, the strip puller including a cathode brush assembly configured to apply a current to the workpiece.
15. The apparatus of claim 9, wherein the plurality of pillars comprises a plurality of perforated riser tubes.
16. An apparatus for continuously electrodepositing a nanolaminate coating on a workpiece, comprising:
  - a. an electrodeposition cell having an anode assembly and a cathode assembly, the anode assembly comprising an anode having a first portion and a second portion that is spaced apart from the first portion, and a plurality of pillars between the first portion and the second portion of the anode, the plurality of pillars arranged in a first

**25**

row and a second row spaced apart from the first row, the pillars having the same dimension along a length of the anode;

a plurality of first rollers that define a path along which the workpiece passes through the electrodeposition cell, the path causing the workpiece not to travel along a center line formed by the first portion and the second portion of the anode, such that a first nanolaminate coating is electrodeposited onto a first surface of the workpiece and a second nanolaminate coating is electrodeposited onto a second surface of the workpiece as the workpiece moves through the electrodeposition cell, the first nanolaminate coating having a first thickness and the second nanolaminate coating having a second thickness that is different than the first thickness;

a power supply electrically connected to the electrodeposition cell, the power supply configured to apply an offset current having three or more different current

5  
10

15

**26**

densities to the workpiece in a time varying manner as the workpiece moves through the electrodeposition cell; and

a strip puller configured to wind the workpiece between the plurality of first rollers, the strip puller including a plurality of second rollers and a cathode brush assembly configured to wind the workpiece between the plurality of second rollers and configured to apply a current to the workpiece, wherein the plurality of second rollers comprises a collection roller around which the workpiece is wound for storage after the nanolaminate coating is electrodeposited.

**17.** The apparatus of claim **16** wherein the path is at a first distance from the first portion of the anode and a second distance from the second portion of the anode, the second distance being different than the first distance.

**18.** The apparatus of claim **16** wherein the path is between the first and second rows of pillars.

\* \* \* \* \*